



US008394746B2

(12) **United States Patent**  
**Carey et al.**

(10) **Patent No.:** **US 8,394,746 B2**  
(b4) **Date of Patent:** **\*Mar. 12, 2013**

(54) **LOW SULFUR AND LOW METAL ADDITIVE FORMULATIONS FOR HIGH PERFORMANCE INDUSTRIAL OILS**

(75) Inventors: **James T. Carey**, Medford, NJ (US); **Angela S. Galiano-Roth**, Mullica Hill, NJ (US); **Margaret M. Wu**, Skillman, NJ (US); **Heather M. Haigh**, Burke, VA (US)

(73) Assignee: **ExxonMobil Research and Engineering Company**, Annandale, NJ (US)

(\*) Notice: Subject to any disclaimer, the term of this patent is extended or adjusted under 35 U.S.C. 154(b) by 642 days.

This patent is subject to a terminal disclaimer.

(21) Appl. No.: **12/583,317**

(22) Filed: **Aug. 18, 2009**

(65) **Prior Publication Data**

US 2010/0048438 A1 Feb. 25, 2010

**Related U.S. Application Data**

(60) Provisional application No. 61/189,766, filed on Aug. 22, 2008.

(51) **Int. Cl.**

**C10M 141/10** (2006.01)  
**C10M 169/04** (2006.01)

(52) **U.S. Cl.** ..... **508/438**; 508/110

(58) **Field of Classification Search** ..... 508/110, 508/438

See application file for complete search history.

(56) **References Cited**

**U.S. PATENT DOCUMENTS**

2,975,442 A 4/1961 Brightbill et al.  
3,149,178 A 9/1964 Hamilton et al.

|             |         |                |
|-------------|---------|----------------|
| 3,164,578 A | 1/1965  | Baker et al.   |
| 3,382,291 A | 5/1968  | Brennan        |
| 3,576,923 A | 4/1971  | Randell et al. |
| 3,742,082 A | 6/1973  | Brennan        |
| 3,769,363 A | 10/1973 | Brennan        |
| 3,780,128 A | 12/1973 | Shubkin        |
| 3,876,720 A | 4/1975  | Heilman et al. |
| 3,883,417 A | 5/1975  | Woo et al.     |
| 4,016,349 A | 4/1977  | McKenna        |
| 4,132,663 A | 1/1979  | Heilman et al. |
| 4,172,855 A | 10/1979 | Shubkin et al. |

(Continued)

**FOREIGN PATENT DOCUMENTS**

|    |            |        |
|----|------------|--------|
| EP | 0119069 A2 | 9/1984 |
| EP | 0119792 A1 | 9/1984 |
| EP | 0088453 B1 | 5/1987 |
| EP | 0276320 B1 | 8/1988 |

(Continued)

**OTHER PUBLICATIONS**

J. Brennan, "Wide-Temperature Range Synthetic Hydrocarbon Fluids", Ind. Eng. Chem. Prod. Res. Dev., 1980, vol. 19, pp. 2-6.

(Continued)

*Primary Examiner* — Walter D Griffin

*Assistant Examiner* — Francis C Campanell

(74) *Attorney, Agent, or Firm* — Robert A. Migliorini

(57) **ABSTRACT**

An additive package, lubricant formulation with the additive package and method of improving gear lubricant properties with the additive package are disclosed. The additive package comprises at least one antiwear additive, at least one antioxidant additive, at least one rust inhibitor additive, at least one metal passivator additive, at least one demulsifier additive, at least one defoamant additive wherein the composition has less than 3.5% phosphorous, less than 1.7% ppm nitrogen, less than 1000 ppm sulfur, less than 100 ppm metals and a TAN of less than 1.

**11 Claims, 4 Drawing Sheets**



## U.S. PATENT DOCUMENTS

|             |         |                      |                  |         |                    |
|-------------|---------|----------------------|------------------|---------|--------------------|
| 4,234,435 A | 11/1980 | Meinhardt et al.     | 5,859,159 A      | 1/1999  | Rossi et al.       |
| 4,239,930 A | 12/1980 | Allphin et al.       | 6,043,401 A      | 3/2000  | Bagheri et al.     |
| 4,263,150 A | 4/1981  | Clason et al.        | 6,080,301 A      | 6/2000  | Berlowitz et al.   |
| 4,263,465 A | 4/1981  | Sheng et al.         | 6,087,307 A      | 7/2000  | Kaminski et al.    |
| 4,289,635 A | 9/1981  | Schroeck             | 6,090,989 A      | 7/2000  | Trewella et al.    |
| 4,308,154 A | 12/1981 | Clason et al.        | 6,133,209 A      | 10/2000 | Rath et al.        |
| 4,367,352 A | 1/1983  | Watts, Jr. et al.    | 6,147,271 A      | 11/2000 | Strebel et al.     |
| 4,413,156 A | 11/1983 | Watts, Jr. et al.    | 6,165,949 A      | 12/2000 | Berlowitz et al.   |
| 4,417,990 A | 11/1983 | Clason et al.        | 6,180,575 B1     | 1/2001  | Nipe               |
| 4,434,308 A | 2/1984  | Larkin et al.        | 6,184,186 B1     | 2/2001  | Ryan et al.        |
| 4,451,684 A | 5/1984  | Pasky                | 6,388,032 B1     | 5/2002  | Yamaura et al.     |
| 4,469,912 A | 9/1984  | Blewett et al.       | 6,395,948 B1     | 5/2002  | Hope et al.        |
| 4,587,368 A | 5/1986  | Pratt                | 6,414,090 B2     | 7/2002  | Minami et al.      |
| 4,652,416 A | 3/1987  | Millot               | 6,479,722 B1     | 11/2002 | De Wet et al.      |
| 4,701,489 A | 10/1987 | Hughes et al.        | 6,548,723 B2     | 4/2003  | Bagheri et al.     |
| 4,704,491 A | 11/1987 | Tsutsui et al.       | 6,548,724 B2     | 4/2003  | Bagheri et al.     |
| 4,776,967 A | 10/1988 | Ichihashi et al.     | 6,589,920 B2     | 7/2003  | Okada et al.       |
| 4,827,064 A | 5/1989  | Wu                   | 6,642,169 B2     | 11/2003 | Weatherhead        |
| 4,827,073 A | 5/1989  | Wu                   | 6,646,174 B2     | 11/2003 | Clarembeau         |
| 4,892,851 A | 1/1990  | Ewen et al.          | 6,706,828 B2     | 3/2004  | DiMaio             |
| 4,906,799 A | 3/1990  | Forbus, Jr. et al.   | 6,713,438 B1     | 3/2004  | Baillargeon et al. |
| 4,910,355 A | 3/1990  | Shubkin et al.       | 6,824,671 B2     | 11/2004 | Goze et al.        |
| 4,912,272 A | 3/1990  | Wu                   | 6,858,767 B1     | 2/2005  | DiMaio et al.      |
| 4,914,254 A | 4/1990  | Pelrine              | 6,869,917 B2     | 3/2005  | Deckman et al.     |
| 4,922,046 A | 5/1990  | Kinoshita et al.     | 7,022,784 B2     | 4/2006  | Wu et al.          |
| 4,926,004 A | 5/1990  | Pelrine et al.       | 7,045,055 B2     | 5/2006  | Ziemer et al.      |
| 4,943,383 A | 7/1990  | Avery et al.         | 7,060,768 B2     | 6/2006  | Brookhart et al.   |
| 4,950,822 A | 8/1990  | Dileo et al.         | 7,129,197 B2     | 10/2006 | Song et al.        |
| 4,956,122 A | 9/1990  | Watts et al.         | 7,312,185 B2     | 12/2007 | Willey et al.      |
| 4,962,249 A | 10/1990 | Chen et al.          | 7,544,850 B2     | 6/2009  | Goze et al.        |
| 4,962,262 A | 10/1990 | Winter et al.        | 7,547,811 B2     | 6/2009  | Kramer et al.      |
| 4,967,032 A | 10/1990 | Ho et al.            | 7,585,823 B2     | 9/2009  | Deckman et al.     |
| 4,990,709 A | 2/1991  | Wu                   | 7,592,411 B2     | 9/2009  | Sullivan et al.    |
| 4,990,711 A | 2/1991  | Chen et al.          | 7,592,497 B2     | 9/2009  | Wu et al.          |
| 5,012,020 A | 4/1991  | Jackson et al.       | 7,683,013 B2     | 3/2010  | Yang et al.        |
| 5,017,299 A | 5/1991  | Gutierrez et al.     | 7,795,194 B2     | 9/2010  | Yang et al.        |
| 5,017,714 A | 5/1991  | Welborn, Jr.         | 2001/0041817 A1  | 11/2001 | Carey et al.       |
| 5,057,235 A | 10/1991 | Farng et al.         | 2001/0041818 A1  | 11/2001 | Bagheri et al.     |
| 5,068,487 A | 11/1991 | Theriot              | 2002/0144853 A1  | 10/2002 | Bagheri et al.     |
| 5,087,788 A | 2/1992  | Wu                   | 2003/0013623 A1  | 1/2003  | Tse et al.         |
| 5,104,579 A | 4/1992  | Benjamin et al.      | 2003/0055184 A1  | 3/2003  | Song et al.        |
| 5,105,038 A | 4/1992  | Chen et al.          | 2003/0092585 A1  | 5/2003  | O'Connor et al.    |
| 5,113,030 A | 5/1992  | Chen et al.          | 2003/0158055 A1  | 8/2003  | Deckman et al.     |
| 5,132,478 A | 7/1992  | Ho et al.            | 2003/0207775 A1  | 11/2003 | Sullivan et al.    |
| 5,146,021 A | 9/1992  | Jackson et al.       | 2003/0236177 A1  | 12/2003 | Wu et al.          |
| 5,157,177 A | 10/1992 | Pelrine et al.       | 2004/0002429 A1  | 1/2004  | Forbus, Jr.        |
| 5,177,276 A | 1/1993  | Beach et al.         | 2004/0029747 A1  | 2/2004  | Emert et al.       |
| 5,180,865 A | 1/1993  | Heilman et al.       | 2004/0033908 A1  | 2/2004  | Blackborow et al.  |
| 5,186,851 A | 2/1993  | Gutierrez et al.     | 2004/0087746 A1  | 5/2004  | Deckman et al.     |
| 5,187,250 A | 2/1993  | Asanuma et al.       | 2004/0147693 A1  | 7/2004  | DiMaio             |
| 5,188,724 A | 2/1993  | Heilman et al.       | 2004/0214733 A1  | 10/2004 | Goze et al.        |
| 5,188,746 A | 2/1993  | Davis                | 2004/0220359 A1  | 11/2004 | Baba               |
| 5,190,682 A | 3/1993  | Harris               | 2004/0225088 A1  | 11/2004 | Abhari et al.      |
| 5,208,403 A | 5/1993  | Buchanan et al.      | 2004/0230016 A1  | 11/2004 | Vaughan et al.     |
| 5,220,100 A | 6/1993  | Massie et al.        | 2005/0059563 A1  | 3/2005  | Blackborow et al.  |
| 5,243,114 A | 9/1993  | Johnson et al.       | 2005/0101761 A1  | 5/2005  | Sullivan et al.    |
| 5,254,274 A | 10/1993 | Ho et al.            | 2005/0113621 A1  | 5/2005  | Lambert et al.     |
| 5,264,642 A | 11/1993 | Wu                   | 2005/0124509 A1  | 6/2005  | Hope et al.        |
| 5,275,749 A | 1/1994  | Kugel et al.         | 2005/0183988 A1  | 8/2005  | Gutierrez et al.   |
| 5,276,227 A | 1/1994  | Wu et al.            | 2005/0250657 A1  | 11/2005 | Freerks et al.     |
| 5,276,277 A | 1/1994  | Hightower et al.     | 2006/0116300 A1  | 6/2006  | Wu et al.          |
| 5,315,053 A | 5/1994  | Beach et al.         | 2006/0116303 A1  | 6/2006  | Arrowsmith et al.  |
| 5,369,196 A | 11/1994 | Matsumoto et al.     | 2006/0122073 A1  | 6/2006  | Iimura et al.      |
| 5,382,739 A | 1/1995  | Atkins et al.        | 2006/0131210 A1  | 6/2006  | Hewette            |
| 5,436,379 A | 7/1995  | Heilman et al.       | 2006/0157383 A1  | 6/2006  | Rosenbaum et al.   |
| 5,462,995 A | 10/1995 | Hosaka et al.        | 2006/0178279 A1  | 7/2006  | Haigh et al.       |
| 5,498,815 A | 3/1996  | Schaerfl, Jr. et al. | 2006/0270568 A1  | 8/2006  | Sullivan et al.    |
| 5,602,086 A | 2/1997  | Le et al.            | 2007/000807 A1   | 1/2007  | Okada et al.       |
| 5,679,812 A | 10/1997 | Winter et al.        | 2007/0043248 A1  | 2/2007  | Haigh et al.       |
| 5,688,887 A | 11/1997 | Bagheri et al.       | 2007/0208151 A1  | 9/2007  | Wu et al.          |
| 5,705,577 A | 1/1998  | Rossi et al.         | 2007/0289897 A1  | 12/2007 | Haigh et al.       |
| 5,731,254 A | 3/1998  | Winter et al.        | 2007/0298990 A1* | 12/2007 | Haigh et al.       |
| 5,807,949 A | 9/1998  | Rossi et al.         | 2008/0020954 A1  | 1/2008  | Haigh et al.       |
| 5,811,379 A | 9/1998  | Rossi et al.         | 2008/0177121 A1  | 7/2008  | Haigh et al.       |
| 5,817,605 A | 10/1998 | Papay                | 2008/0207475 A1  | 8/2008  | Haigh et al.       |
| 5,846,896 A | 12/1998 | Ewen                 | 2009/0005279 A1  | 1/2009  | Haigh et al.       |
| 5,852,143 A | 12/1998 | Sishta et al.        |                  |         | ..... 508/591      |
| 5,858,935 A | 1/1999  | Watts et al.         |                  |         |                    |

2009/0036725 A1 2/2009 Wu et al.  
 2009/0093657 A1 4/2009 Buchanan et al.  
 2009/0156874 A1 6/2009 Patil et al.  
 2009/0240012 A1 9/2009 Patil et al.  
 2010/0006259 A1 1/2010 Mori et al.  
 2010/0256026 A1 10/2010 Wu et al.  
 2010/0292424 A1 11/2010 Wu et al.  
 2011/0082063 A1 4/2011 Carey et al.  
 2011/0136714 A1 6/2011 Haigh et al.

## FOREIGN PATENT DOCUMENTS

EP 0277004 A1 8/1988  
 EP 0277007 B1 8/1988  
 EP 0284708 B1 10/1988  
 EP 0291006 B1 11/1988  
 EP 0321852 B1 6/1989  
 EP 0349276 B1 1/1990  
 EP 0377306 B1 7/1990  
 EP 0403866 A1 12/1990  
 EP 0513380 B1 11/1992  
 EP 0680942 A1 5/1994  
 EP 0613873 A2 9/1994  
 EP 0930320 A1 7/1997  
 EP 1028128 A1 10/1997  
 EP 0992517 A2 9/1998  
 EP 1309633 B1 8/2000  
 EP 1308496 B1 5/2003  
 EP 1342707 A2 9/2003  
 EP 1607415 A1 12/2005  
 EP 1661921 A1 5/2006  
 GB 938069 9/1963  
 IN 191553 12/2003  
 JP 6336590 A 12/1994  
 JP 200500446 A 7/2005  
 WO 9623751 8/1996  
 WO 9804658 2/1998  
 WO 9967347 6/1999  
 WO 0058423 10/2000  
 WO 0214384 A2 2/2002  
 WO 03009136 A1 1/2003  
 WO 03020856 A1 3/2003  
 WO 03051943 A1 6/2003  
 WO 03071369 A1 8/2003  
 WO 03104292 A1 12/2003  
 WO 2004046214 A2 6/2004  
 WO 2004053030 A2 6/2004  
 WO 2005111178 A1 12/2005  
 WO 2006071595 A2 7/2006  
 WO 2006083632 A1 8/2006  
 WO 2007005094 A1 1/2007  
 WO 2007011832 A1 1/2007  
 WO PCT/WO2007/011459 A1 1/2007  
 WO PCT/WO2007/011462 A1 1/2007  
 WO 2007145924 A1 12/2007  
 WO 2007146081 A1 12/2007  
 WO 2008010865 A2 1/2008  
 WO 2009017953 A2 2/2009  
 WO 2009123800 A1 10/2009  
 WO 2009137264 A1 11/2009

## OTHER PUBLICATIONS

K. Denbigh, "The Kinetics of Continuous Reaction Processes: Application to Polymerization", *J. Applied Chem.*, 1951, vol. 1, pp. 227-236.

K. Denbigh, "Continuous Reactions: Part II. The Kinetics of Steady State Polymerisation", *Trans Faraday Soc.*, 1947, vol. 43, pp. 648-660.

A. Munoz-Escalona, et al., "Single-Site Supported Catalysts for Ethylene Polymerization", *Metallocene Tech.*, 1999, pp. 2242-2246.

Z. Fan, et al., "Effect of Ethoxy- and Methoxysilane Donors in Propene/1-Hexene Copolymerization with High-Yield Supported Ziegler-Natta Catalysts", *Macromolecular Chemistry and Physics*, 1994, vol. 195, pp. 3889-3899.

G. Gokel, ed., "Dean's Handbook of Organic Chemistry", 2nd Edition, McGraw-Hill, 2004, available on-line at <http://knovel.com>.

M. LeVan, et al., "Adsorption and Ion Exchange", *Perry's Chemical Engineer's Handbook*, 7th ed., 1997, pp. 16-1-16-66.

O. Levenspiel, "Ch. 7: Design for Multiple Reactions", *Chemical Reaction Engineering*, 2nd ed., 1972, pp. 196-209.

N. Naga, et al., "Effect of Co-Catalyst System on a-Olefin Polymerization with Rac- and Meso-[Dimethylsilylenebis (2,3,5-Trimethyl-Cyclopentadienyl)] Zirconium Dichloride", *Macromol. Rapid Commun.*, 1997, vol. 18, pp. 581-589.

N. Naga, et al., "Polymerization Behavior of a-Olefins with Rac- and Meso-Type Ansa-Metallocene Catalyst: Effects of Cocatalyst and Metallocene Ligand", *Macromolecular Chemistry Physics*, 1999, vol. 200, pp. 1587-1594.

F. Rodriguez, "The Molecular Weight of Polymers", *Principles of Polymer Systems*, 1970, Chapter 6, pp. 115-144.

M. Sacchi, et al., "Use of Different Alkoxy silanes as External Donors in MgCl<sub>2</sub>-Supported Ziegler-Natta Catalysts to Obtain Propene/1-Butene Copolymers with Different Microstructure", *Macromolecular Chemistry and Physics*, 1994, vol. 195, pp. 2805-2816.

T. Seraidaris, et al., "High-Molar-Mass Polypropene with Tunable Elastic Properties by Hafnocene/Borate Catalysts", *Journal of Polymer Science: Part A: Polymer Chemistry*, 2006, vol. 44, pp. 4743-4751.

J. Wills, "Synthetic Lubricants", *Lubrication Fundamentals*, Marcel Dekker Inc., New York, 1980, pp. 75-80.

"Mobil Releases SuperSyn PAO's", *Lubrication Engineers*, 1999, vol. 55, Part 8, pp. 45.

TIBA data, "TIBA datasheet" available on-line at [www.albermarle.com](http://www.albermarle.com) on Aug. 26, 2010.

ASTM D3427-03, "Standard Test Method for Air Release Properties of Petroleum Oils", Oct. 2002.

<http://www.mobil.com/USA>, Mobilgear® SHC XMP Series, Jun. 2005.

[http://www.famm11c.com/famm/lubricant\\_product.asp?gearoils&&wPinnacleMarineGear220](http://www.famm11c.com/famm/lubricant_product.asp?gearoils&&wPinnacleMarineGear220), Pinnacle® Marine Gear 220, Nov. 2007.

Rudnick, Leslie R., "Synthetics, Mineral Oils, and Bio-Based Lubricants Chemistry and Technology", published by CRC Press, Taylor & Francis Group, 2006, 37-46.

Corsico, G. et al., "Poly(intemal olefins)", *EURON*, Milan, Italy, Chemical Industries (Dekker), 1999, 77(Synthetic Lubricants and High-Performance Functional Fluids, 2<sup>nd</sup> Edition, 53-62.

Kirk-Othmer Encyclopedia of Chemical Technology, Second completely revised edition, "Diamines and Higher Amines, Aliphatic", vol. 7, 1965, published by John Wiley & Sons, Inc., 22-39.

\* cited by examiner

Figure 1



Figure 2



**Figure 3**  
**Performance Benefits in Worm Gears: % Efficiency**



**Figure 4**  
**Operating Temperature : Degrees F**



## 1

**LOW SULFUR AND LOW METAL ADDITIVE  
FORMULATIONS FOR HIGH  
PERFORMANCE INDUSTRIAL OILS**

**CROSS-REFERENCE TO RELATED  
APPLICATION(S)**

Non Provisional Application based on U.S. Ser. No. 61/189,766 filed Aug. 22, 2008.

**BACKGROUND**

The lubrication of industrial equipment including gears and enclosed gearboxes has become increasingly more difficult. This difficulty is partially caused by machinery builders continually shrinking equipment and driving more power through a given speed reducer. Generally, gear oil consists of base oil more viscous than typical engine oils, and an additive package which is formulated to enhance various performance features. These additive features include: protection against wear, resistance to thickening by the use of antioxidants, rust protection, copper-metal passivation, demulsification, air release and foam control amongst others. Industrial gear oils have to achieve the following requirements: excellent resistance to aging and oxidation, low foaming tendency, good load-carrying capacity, neutrality toward the materials involved (ferrous and nonferrous metals, seals, paints), suitability for high and/or low temperatures, and good viscosity-temperature behavior.

The most important performance feature that additives impart is antiwear protection. The most prevalent antiwear additive systems in lubricating gears oils contain combinations of sulfur-containing hydrocarbons with various amine-phosphates, and/or phosphates. The key downside of these sulfur-containing additives is that while they protect against wear, they do rapidly hydrolyze in the presence of acidic contaminants. This reaction produces sulfuric acid, causing excessive corrosive damage. It is then very desirable to develop gear oil which is capable of delivering all the previous mentioned features while being sulfur free or at least low sulfur.

Oil operating temperature & efficiencies are very important to the designers, builders, and user of equipment which employ worm gearing. On a relative basis, a higher percentage efficiency rating for a lubricant results in more power (torque) being transmitted through a subject gearbox. Since more power is being transferred through a piece of equipment using a more efficient lubricant, less power is being wasted to friction or heat. It is desirable for a lubricant to be optimized for maximum power throughput and to therefore allow for lower operating temperatures. Lower operating temperatures in gearboxes give rise to several benefits which include: lower energy consumption, longer machine life, and longer seal life. Seal failures are one of the principle reasons for repair and down-time in rotating equipment. A decrease of 10 degrees Celsius of operating temperature can double seal life and therefore decrease overall costs of operation and ownership.

A Small Worm Gear Rig ("SWGR") measures both dynamic operating temperature and efficiency of power throughput simultaneously. In this SWGR gear rig, a splash lubricated bronze on steel worm gear set is the gearbox design employed. The subject worm drive gearbox with a 1.75 inch centerline distance, 20:1 reduction ratio, was mounted in an L-shaped test rig with high precision torque meters on both the input and output shafts of the gearbox to measure power throughput efficiency performance based on control of output torque. The output torque was controlled to 100% of the rated

## 2

load with a service factor of 1.0. Also, gearbox sump oil temperature was carefully monitored during operation using four thermocouples. National Basic Sensor located at 4921 Carver Avenue in Trevose, Pa. sells J-type thermocouples that are suitable for this rig test.

All torque and temperature data was logged every 10 seconds for a period of 12 hours after thermal stability was attained. The efficiency was calculated by establishing the ratio of output torque to input torque. The resulting efficiency and operational temperatures compare experimental blends against reference oils.

In addition to temperature and efficiency, air entrainment is another issue in lubricating oils. All lubricating oil systems contain some air. It can be found in four phases: free air, dissolved air, entrained air and foam. Free air is trapped in a system, such as an air pocket in a hydraulic line. Dissolved air is in solution with the oil and is not visible to the naked eye. Foam is a collection of closely packed bubbles surrounded by thin films of oil that collect on the surface of the oil.

Air entrainment is a small amount of air in the form of extremely small bubbles (generally less than 1 mm in diameter) dispersed throughout the bulk of the oil. Agitation of lubricating oil with air in equipment, such as bearings, couplings, gears, pumps, and oil return lines, may produce a dispersion of finely divided air bubbles in the oil. If the residence time in the reservoir is too short to allow the air bubbles to rise to the oil surface, a mixture of air and oil will circulate through the lubricating oil system. This may result in an inability to maintain oil pressure (particularly with centrifugal pumps), incomplete oil films in bearings and gears, and poor hydraulic system performance or failure. Air entrainment is treated differently than foam, and is most often a completely separate problem. A partial list of potential effects of air entrainment include: pump cavitation, spongy, erratic operation of hydraulics, loss of precision control; vibrations, oil oxidation, component wear due to reduced lubricant viscosity, equipment shut down when low oil pressure switches trip, "micro-dieseling" due to ignition of the bubble sheath at the high temperatures generated by compressed air bubbles, safety problems in turbines if overspeed devices do not react quickly enough, and loss of head in centrifugal pumps.

Antifoamants, including silicone additives help produce smaller bubbles in the bulk of the oil. In stagnant systems, the combination of smaller bubbles and greater sheath density can cause serious air entrainment problems. Turbine oil systems with quiescent reservoirs of several thousand gallons may have air entrainment problems with as little as a half a part per million silicone.

One widely used method to test air release properties of petroleum oils is ASTM D3427-03. This test method measures the time for the entrained air content to fall to the relatively low value of 0.2% under a standardized set of test conditions and hence permits the comparison of the ability of oils to separate entrained air under conditions where a separation time is available. The significance of this test method has not been fully established. However, entrained air can cause sponginess and lack of sensitivity of the control of turbine and hydraulic systems. This test may not be suitable for ranking oils in applications where residence times are short and gas contents are high.

In the ASTM D3427 method, compressed air is blown through the test oil, which has been heated to a temperature of 25, 50, or 75° C. After the air flow is stopped, the time required for the air entrained in the oil to reduce in volume to 0.2% is usually recorded as the air release time.

A universal industrial oil lubricant with low sulfur and low metals and providing favorable performance properties is not commercially available. Accordingly, there is a need for an additive package and lubricant formulation that provides a consistent favorable operating temperature and power efficiency along with air release properties using high viscosity base stock blends. The present invention satisfies this need by providing a novel combination of additives that give the desired performance.

## SUMMARY

A novel additive package for industrial lubricants is disclosed. The additive package comprises at least one antiwear additive, at least one antioxidant additive, at least one rust inhibitor additive, at least one metal passivator additive, at least one demulsifier additive, at least one defoamant additive wherein the composition has less than 3.50% phosphorous, less than 1.70% nitrogen, less than 1000 ppm sulfur, less than 100 ppm metals and a total acid number ("TAN") of less than 1.0.

In a second embodiment, a novel lubricant formulation is disclosed. This lubricant formulation comprises at a first base stock PAO with a viscosity at least 100 cSt, Kv100° C.; a second base stock comprising a oil with a viscosity less than 40 cSt, Kv100° C.; a third basestock comprising low viscosity co-base oil selected from the group consisting of Ester, alkylated aromatic, and any combination thereof; an additive package comprising at least one antiwear additive, at least one antioxidant additive, at least one rust inhibitor additive, at least one metal passivator additive, at least one demulsifier additive, at least one defoamant additive; wherein the composition has less than 1000 ppm phosphorous, less than 300 ppm nitrogen, 10 ppm metals, less than 30 ppm sulfur and a tan of less than 1.

A method for achieving favorable gear lubrication is disclosed. This method comprises obtaining a obtaining a first synthetic base stock lubricant the first base stock having a viscosity greater than 100 cSt, Kv100° C. and the first bases stock having a molecular weight distribution (MWD) as a function of viscosity at least 10 percent less than algorithm:  $MWD=0.2223+1.0232*\log(Kv \text{ at } 100^\circ \text{ C. in cSt})$ ; obtaining a second synthetic base stock lubricant, the second base stock lubricant has a viscosity less than 60 cSt, Kv100° C.; obtaining an additive package comprising at least one antiwear additive, at least one antioxidant additive, at least one rust inhibitor additive, at least one metal passivator additive, at least one demulsifier additive, at least one defoamant additive; blending the first base stock, the second base stock and additive package to formulate the lubricating oil.

## BRIEF DESCRIPTION OF THE DRAWINGS

FIG. 1 is a graph illustrating the molecular weight distribution of high viscosities PAO;

FIG. 2 is a graph illustrating the improved viscosities losses or improved shear stability as a function of the viscosity of the high viscosity metallocene catalyzed base stocks;

FIG. 3 is a graph showing the improved SWGR efficiency of gear oils formulated with the low sulfur, low metal additive packages when compared to a commercially available gear oil package blended with the same base stock formulation;

FIG. 4 is a graph showing the improved SWGR operating temperature of gear oils formulated with the low sulfur, low metal additive packages when compared to a commercially available gear oil package blended with the same base stock formulation.

## DETAILED DESCRIPTION

In another embodiment, we have discovered an improved additive package. In one embodiment, this additive package has low levels of sulfur and metals. This additive package will work well with all base stocks. However, Applicants have discovered there are additional synergistic benefits when the additives are used in bi-modal blend of metallocene catalyzed PAO.

In this patent, unless specified otherwise, all base stock viscosities are referred to their 100° C. kinematics viscosity in cSt as measured by ASTM D445 method. The ISO viscosity classification which is typically cited for industrial lubes of finished lubricants is based on viscosities observed at 40° C. In a preferred embodiment, we have discovered novel combinations of base stocks with an additive package that provide unexpected favorable improvements in lubricating properties. In various embodiments these properties include favorable improvements in shear stability, air release, pour point, temperature control, viscosity loss and energy efficiency. In U.S. Provisional Application No. 60/811,273, we have discovered a novel combination of base stocks that provides an unexpected increase in aeration properties, shear stability and energy efficiency. In U.S. Provisional Application No. 60/811,207, we have discovered the benefits of using metallocene catalyzed PAO compared to the prior art PAO.

In this preferred embodiment, the inventors have discovered a lubricant which is directed to oil and grease formulations for industrial oils. This lubricant comprises a polyalphaolefin (PAO) in combination with various groups III and other PAO's, a polar co-basestock, and an optimized additive system which contains no sulfur or metal containing additives.

In one embodiment, the additive package comprises at least one antiwear additive, at least one rust inhibitor, at least one friction modifier, at least one metal passivator, at least one antioxidant, and at least one defoamant which may or may not include a demulsifier. In a preferred embodiment the antiwear is a phosphate or amine phosphate. The rust inhibitor is an alkylated acid type. The friction modifier is a phosphonate, the metal passivator is an amine phosphate and the defoamant and/or demulsifier is an antifoam package.

In more preferred embodiments, the additive formulations according to the present invention are used in combination with base stocks as fully formulated gear oils, circulating oils, compressors oils, hydraulic oils, refrigeration lubes, metalworking fluids and greases. More specific embodiments give rise to gear oil lubricants which provide high viscosity indexes, excellent air release properties, and good low temperature performance. Most specifically, a VI greater than 170, air release less than 10 minutes in the ASTM D3427 test, and pour points less than -30° C. are desirable without VI improvers.

Table 1 lists the preferred more preferred and most preferred ranges of the types of additives used in this embodiment. The ranges are given in weight percent of the total additive concentration. Preferably the additive should have low levels of metal and sulfur. Most preferably the additives have no sulfur and no metal.

TABLE 1

|                  | Preferred wt % | More Preferred wt % | Most Preferred wt % |
|------------------|----------------|---------------------|---------------------|
| Antiwear         | 25-50          | 35-45               | 38-42               |
| Antirust         | 5-15           | 8-12                | 9-11                |
| Metal Passivator | 1-5            | 2-4                 | 2.5-3.5             |

TABLE 1-continued

|                   | Preferred wt % | More Preferred wt % | Most Preferred wt % |
|-------------------|----------------|---------------------|---------------------|
| Antioxidant       | 10-20          | 12-17               | 13-15               |
| Friction Modifier | 10-30          | 15-26               | 20-25               |
| Defoamant         | 3-10           | 4-8                 | 5-7                 |

Table 2 illustrates the preferred base stock combinations with preferred ranges, more preferred and most preferred component ranges. In the preferred embodiment there are at least three base stock components including a high viscosity base stock of at least 100 cST KV 100° C., a low viscosity

base stock component of less than 10 cST KV 100° C., and a low viscosity co-base stock oil.

In this preferred embodiment the high viscosity base stock is selected from the group consisting of metallocene catalyzed PAO with a viscosity of at least 100, a PAO with a viscosity less than 10 and any combination thereof. The low viscosity base stock is selected from the group consisting of PAO, GTL and Visom, metallocene catalyzed PAO with a viscosity of at least 150, a PAO with a viscosity at least 100 and any combination thereof. The low viscosity co-base stock oil is selected from the group consisting Adipate ester, TMP Ester, Alkylated Napthylene, Phthalate ester, and any combination thereof.

TABLE 2

| Description               | Specific Type         | Ranges (Wt %) |                |                       | Viscosity                    |                               |
|---------------------------|-----------------------|---------------|----------------|-----------------------|------------------------------|-------------------------------|
|                           |                       | Preferred     | More Preferred | Most Preferred (Best) | KV 40° C. mm <sup>2</sup> /s | KV 100° C. mm <sup>2</sup> /s |
| High Viscosity Base oil   | m150                  | 1.00-90.00    | 20.00-70.00    | 35.00-60.00           | 1719                         | 157.6                         |
| High Viscosity Base oil   | PAO 100               | 1.00-90.00    | 20.00-70.00    | 35.00-60.00           | 1250                         | 100                           |
| Low Viscosity Base oil    | PAO 4                 | 5.00-50.00    | 10.00-20.00    | 12.00-18.00           | 18.0                         | 4.1                           |
| Low Viscosity Base oil    | Visom 4               | 5.00-50.00    | 10.00-20.00    | 12.00-18.00           | 16.8                         | 4.0                           |
| Low Viscosity Base oil    | GTL 4                 | 5.00-50.00    | 10.00-20.00    | 12.00-18.00           | 16.8                         | 4.0                           |
| Low Viscosity Co-Base oil | Adipate ester         | 5.00-20.00    | 8.00-15.00     | 10.00-14.00           | 26.8                         | 5.2                           |
| Low Viscosity Co-Base oil | TMP Ester             | 5.00-20.00    | 8.00-15.00     | 10.00-14.00           | 25.9                         | 4.9                           |
| Low Viscosity Co-Base oil | Alkylated Naphthalene | 5.00-20.00    | 8.00-15.00     | 10.00-14.00           | 29.3                         | 4.7                           |
| Low Viscosity Co-Base oil | Phthalate ester       | 5.00-20.00    | 8.00-15.00     | 10.00-14.00           | 83                           | 12.2                          |

The preferred additive is listed in table 2. The ranges given are for fully formulated lubricant oil. The additives would work in any base stocks but are preferably designed for the base stocks combinations listed in Table 1.

TABLE 3

| Additive Function | Description         | Ranges (WT %) |                | Ranges (WT %) | Viscosity                    |                               |
|-------------------|---------------------|---------------|----------------|---------------|------------------------------|-------------------------------|
|                   |                     | Preferred     | More Preferred |               | KV 40° C. mm <sup>2</sup> /s | KV 100° C. mm <sup>2</sup> /s |
| Antiwear          | Phosphate           | 0.05-1.00     | 0.10-0.50      | 0.15-0.45     | 15.4                         | —                             |
| Antiwear          | Amine               | 0.05-0.50     | 0.10-0.40      | 0.15-0.35     | 2489                         | 75.0                          |
| Rust Inhibitor    | Phosphate           | 0.05-0.50     | 0.10-0.40      | 0.15-0.35     | 1750                         | 32                            |
| Rust Inhibitor    | Alkylated Acid type | 0.05-0.50     | 0.10-0.40      | 0.15-0.35     | 2500                         | —                             |
| Friction Modifier | Alkylated Acid type | 0.05-0.50     | 0.10-0.30      | 0.15-0.25     | solid                        | 4.0                           |
|                   | Phosphonate         | 0.05-0.60     | 0.10-0.40      | 0.15-0.35     |                              |                               |

TABLE 3-continued

| Additive Function      | Description      | Ranges (WT %) |                | Ranges (WT %) | Most Preferred (Best) | Viscosity KV 40° C. mm <sup>2</sup> /s | Viscosity KV 100° C. mm <sup>2</sup> /s |
|------------------------|------------------|---------------|----------------|---------------|-----------------------|----------------------------------------|-----------------------------------------|
|                        |                  | Preferred     | More Preferred |               |                       |                                        |                                         |
| Metal Passivator       | Amine            | 0.01-0.50     | 0.05-0.30      | 0.10-0.20     | 80                    | —                                      | —                                       |
|                        | Phosphate        |               |                |               |                       |                                        |                                         |
| Antioxidant            | Alkylated        | 0.05-1.00     | 0.10-0.80      | 0.3-0.60      | 300                   | —                                      | —                                       |
|                        | Aryl Amine       |               |                |               |                       |                                        |                                         |
| Defoamant/ Demulsifier | Antifoam Package | 0.01-0.50     | 0.10-0.30      | 0.15-0.25     | 2.2                   | —                                      | —                                       |

The table below shows the TAN, and Weight Percentages of Phosphorous, Nitrogen and Sulfur respectively for each additive from Table 2.

15 In one embodiment, this novel discovery is based on wide “bi-modal” and “extreme-modal” blends of oil viscosities which are base stock viscosity differences of at least 60 cSt,

TABLE 4

| Additive Function      | TAN (mgKOH/g) of Neat Component | TAN (mgKOH/g) in Finished oil | Phosphorus (wt %) of Neat Component | Phosphorus (wt %) in Finished oil | Nitrogen (wt %) of Neat Component | Nitrogen (wt %) in Finished oil | Sulfur (wt %) of Neat Component | Sulfur (wt %) in Finished oil |
|------------------------|---------------------------------|-------------------------------|-------------------------------------|-----------------------------------|-----------------------------------|---------------------------------|---------------------------------|-------------------------------|
|                        |                                 |                               |                                     |                                   |                                   |                                 |                                 |                               |
| Antiwear               | 0.1                             | 0.0001                        | 8.9                                 | 0.0089                            | 0.0                               | 0.0                             | 0.0                             | 0.0                           |
| Antiwear               | 200                             | 0.500                         | 3.9                                 | 0.0098                            | NA                                | NA                              | 0.0                             | 0.0                           |
| Rust Inhibitor         | 203                             | 0.2390                        | 0.0                                 | 0.0                               | 0.0                               | 0.0                             | 0.0                             | 0.0                           |
| Rust Inhibitor         | 200                             | 0.6000                        | 0.0                                 | 0.0                               | 0.0                               | 0.0                             | 0.0                             | 0.0                           |
| Friction Modifier      | 0.0                             | 0.0                           | 8.3                                 | 0.0208                            | 0.0                               | 0.0                             | 0.0                             | 0.0                           |
| Metal Passivator       | 0.0                             | 0.0                           | 0.0                                 | 0.0                               | 3.65                              | 0.0037                          | 0.0                             | 0.0                           |
| Antioxidant            | 0.0                             | 0.0                           | 0.0                                 | 0.0                               | 4.50                              | 0.0180                          | 0.0                             | 0.0                           |
| Defoamant/ Demulsifier | 0.0                             | 0.0                           | 0.0                                 | 0.0                               | 0.0                               | 0.0                             | 0.0                             | 0.0                           |
|                        |                                 | 1.19                          |                                     | 0.0385                            |                                   | 0.0394                          | 0.00                            |                               |
|                        |                                 |                               |                                     | 385 ppm                           |                                   | 394 ppm                         | <10 ppm                         |                               |

In one embodiment, the additive combination includes an antiwear additive, an antioxidant additive, an antirust additive, a metal passivator a demulsifier and an antifoam additive. Preferably, the antiwear additive has at least two components at least one phosphate ester and at least one amine phosphate. The antioxidant is preferably an aryl amine, the anti rust additive is preferably a amide carboxylate. The metal passivator is preferably an amine phosphate. The demulsifier is preferably a low molecular weight extreme pressure or EO-PO polymer. The antifoam/defoamant is preferably a two component system with at least one polysiloxanes and at least one polymethacrylate. In addition, an antiwear friction reducer can be added with the preferred additive being an oleyl phosphate.

In one embodiment, the additive package and finished formulations are low metal and low sulfur lubricants. In various embodiments each metal compound of calcium, magnesium, barium, sodium, and potassium should be less than 20 ppm of the lubricant. Molybdenum and zinc should be less than 10 ppm of the lubricant. Preferably the additives should be substantially free of metals. For purposes of this application, substantially free of metals shall be considered less than 1 ppm of any individual metal or an oil with less than 10 ppm content of all metals combined.

In addition the phosphorous should be less than 1000 ppm with a preferred range of greater than 300 and less than 1000 ppm. The nitrogen should be less than 500 ppm. The sulfur should be less than 30 ppm, more preferably less than 20 ppm and most preferably less than 10 ppm. The TAN is preferably less than 1.0, more preferably less than 0.8 and most preferably less than 0.5.

preferably at least 100 cSt, and possibly greater than 250 cSt, respectively wherein the high viscosity is at least 80 cSt, and the low viscosity base stock is less than 60 cSt. Kinematic Viscosity is determined by ASTM D-445 method by measuring the time for a volume of liquid to flow under gravity through a calibrated glass capillary viscometer. Viscosity is typically measured in centistokes (cSt, or mm<sup>2</sup>/s) units. The ISO viscosity classification which is typically cited for industrial lubes of finished lubricants based on viscosities observed at 40° C. Base stock oils used to blend finished oils, are generally described using viscosities observed at 100° C.

40 This “bi-modal” blend of viscosities also provides a temperature benefit by lowering the lubricant temperature in gear testing by approximately 10° C. This temperature drop would 45 provide increased efficiency boosts and extended seal life.

In the past high viscosity base stocks have not been practical from some most applications due to shear stability problems resulting in viscosity loss in service due to breakdown of 50 polymeric chains. We have discovered that new base stocks with low with narrow molecular weight distributions provide excellent shear stability. This discovery provided the ability to utilize high viscosity base stocks in what can be described as “dumbbell”, “bi-modal” and “extreme-modal” blends.

55 In a preferred embodiment, the new base stocks are produced according to the method described in U.S. Provisional Application Nos. 60/650,206. These base stocks are known as metallocene catalyzed bases stocks and are described in detail below.

#### 60 Metallocene Base Stocks

In one embodiment, the metallocene catalyzed PAO (or mPAO) used for this invention can be a co-polymer made

from at least two alpha-olefins or more, or a homo-polymer made from a single alpha-olefin feed by a metallocene catalyst system.

This copolymer mPAO composition is made from at least two alpha-olefins of C3 to C30 range and having monomers randomly distributed in the polymers. It is preferred that the average carbon number is at least 4.1. Advantageously, ethylene and propylene, if present in the feed, are present in the amount of less than 50 wt % individually or preferably less than 50 wt % combined. The copolymers of the invention can be isotactic, atactic, syndiotactic polymers or any other form of appropriate tacticity. These copolymers have useful lubricant properties including excellent VI, pour point, low temperature viscometrics by themselves or as blend fluid with other lubricants or other polymers. Furthermore, these copolymers have narrow molecular weight distributions and excellent lubricating properties.

In an embodiment, mPAO is made from the mixed feed LAOs comprising at least two and up to 26 different linear alpha-olefins selected from C3 to C30 linear alpha-olefins. In a preferred embodiment, the mixed feed LAO is obtained from an ethylene growth process using an aluminum catalyst or a metallocene catalyst. The growth olefins comprise mostly C6 to C18-LAO. LAOs from other process, such as the SHOP process, can also be used.

This homo-polymer mPAO composition is made from single alpha-olefin choosing from C3 to C30 range, preferably C3 to C16, most preferably C3 to C14 or C3 to C12. The homo-polymers of the invention can be isotactic, atactic, syndiotactic polymers or any combination of these tacticity or other form of appropriate tacticity. Often the tacticity can be carefully tailored by the polymerization catalyst and polymerization reaction condition chosen or by the hydrogenation condition chosen. These homo-polymers have useful lubricant properties including excellent VI, pour point, low temperature viscometrics by themselves or as blend fluid with other lubricants or other polymers. Furthermore, these homo-polymers have narrow molecular weight distributions and excellent lubricating properties.

In another embodiment, the alpha-olefin(s) can be chosen from any component from a conventional LAO production facility or from refinery. It can be used alone to make homo-polymer or together with another LAO available from refinery or chemical plant, including propylene, 1-butene, 1-pentene, and the like, or with 1-hexene or 1-octene made from dedicated production facility. In another embodiment, the alpha-olefins can be chosen from the alpha-olefins produced from Fischer-Trosch synthesis (as reported in U.S. Pat. No. 5,382,739). For example, C3 to C16-alpha-olefins, more preferably linear alpha-olefins, are suitable to make homo-polymers. Other combinations, such as C4 and C14-LAO; C6 and C16-LAO; C8, C10, C12-LAO; or C8 and C14-LAO; C6, C10, C14-LAO; C4 and C12-LAO, etc. are suitable to make co-polymers.

The activated metallocene catalyst can be simple metallocenes, substituted metallocenes or bridged metallocene catalysts activated or promoted by, for instance, methylaluminoxane (MAO) or a non-coordinating anion, such as N,N-dimethylalilinium tetrakis(perfluorophenyl)borate or other equivalent non-coordinating anion and optionally with co-activators, typically trialkylaluminum compounds.

According to the invention, a feed comprising a mixture of LAOs selected from C3 to C30 LAOs or a single LAO selected from C3 to C16 LAO, is contacted with an activated metallocene catalyst under oligomerization conditions to provide a liquid product suitable for use in lubricant components or as functional fluids. This invention is also directed to a

copolymer composition made from at least two alpha-olefins of C3 to C30 range and having monomers randomly distributed in the polymers. The phrase "at least two alpha-olefins" will be understood to mean "at least two different alpha-olefins" (and similarly "at least three alpha-olefins" means "at least three different alpha-olefins", and so forth).

In preferred embodiments, the average carbon number (defined hereinbelow) of said at least two alpha-olefins in said feed is at least 4.1. In another preferred embodiment, the amount of ethylene and propylene in said feed is less than 50 wt % individually or preferably less than 50 wt % combined. A still more preferred embodiment comprises a feed having both of the aforementioned preferred embodiments, i.e., a feed having an average carbon number of at least 4.1 and wherein the amount of ethylene and propylene is less than 50 wt % individually.

In embodiments, the product obtained is an essentially random liquid copolymer comprising the at least two alpha-olefins. By "essentially random" is meant that one of ordinary skill in the art would consider the products to be random copolymer. Other characterizations of randomness, some of which are preferred or more preferred, are provided herein. Likewise the term "liquid" will be understood by one of ordinary skill in the art, but more preferred characterizations of the term are provided herein. In describing the products as "comprising" a certain number of alpha-olefins (at least two different alpha-olefins), one of ordinary skill in the art in possession of the present disclosure would understand that what is being described in the polymerization (or oligomerization) product incorporating said certain number of alpha-olefin monomers. In other words, it is the product obtained by polymerizing or oligomerizing said certain number of alpha-olefin monomers.

This improved process employs a catalyst system comprising a metallocene compound (Formula 1, below) together with an activator such as a non-coordinating anion (NCA) (Formula 2, below) and optionally a co-activator such as a trialkylaluminum, or with methylaluminoxane (MAO) (Formula 3, below).



Formula 1



Formula 2



Formula 3

The term "catalyst system" is defined herein to mean a catalyst precursor/activator pair, such as a metallocene/activator pair. When "catalyst system" is used to describe such a pair before activation, it means the unactivated catalyst (pre-catalyst) together with an activator and, optionally, a co-activator (such as a trialkyl aluminum compound). When it is used to describe such a pair after activation, it means the

## 11

activated catalyst and the activator or other charge-balancing moiety. Furthermore, this activated “catalyst system” may optionally comprise the co-activator and/or other charge-balancing moiety. Optionally and often, the co-activator, such as trialkylaluminum compound, is also used as impurity scavenger.

The metallocene is selected from one or more compounds according to Formula 1, above. In Formula 1, M is selected from Group 4 transition metals, preferably zirconium (Zr), hafnium (Hf) and titanium (Ti), L1 and L2 are independently selected from cyclopentadienyl (“Cp”), indenyl, and fluorenyl, which may be substituted or unsubstituted, and which may be partially hydrogenated, A can be no atom, as in many un-bridged metallocenes or A is an optional bridging group which if present, in preferred embodiments is selected from dialkylsilyl, dialkylmethyl, diphenylsilyl or diphenylmethyl, ethylenyl ( $-\text{CH}_2-\text{CH}_2-$ ), alkylethylenyl ( $-\text{CR}_2-\text{CH}_2-$ ), where alkyl can be independently C1 to C16 alkyl radical or phenyl, tolyl, xylyl radical and the like, and wherein each of the two X groups, Xa and Xb, are independently selected from halides, OR (R is an alkyl group, preferably selected from C1 to C5 straight or branched chain alkyl groups), hydrogen, C1 to C16 alkyl or aryl groups, haloalkyl, and the like. Usually relatively more highly substituted metallocenes give higher catalyst productivity and wider product viscosity ranges and are thus often more preferred.

In another embodiment, any of the polyalpha-olefins produced herein preferably have a Bromine number of 1.8 or less as measured by ASTM D 1159, preferably 1.7 or less, preferably 1.6 or less, preferably 1.5 or less, preferably 1.4 or less, preferably 1.3 or less, preferably 1.2 or less, preferably 1.1 or less, preferably 1.0 or less, preferably 0.5 or less, preferably 0.1 or less.

In another embodiment, any of the polyalpha-olefins produced herein are hydrogenated and have a Bromine number of 1.8 or less as measured by ASTM D 1159, preferably 1.7 or less, preferably 1.6 or less, preferably 1.5 or less, preferably 1.4 or less, preferably 1.3 or less, preferably 1.2 or less, preferably 1.1 or less, preferably 1.0 or less, preferably 0.5 or less, preferably 0.1 or less.

In another embodiment, any of the polyalpha-olefins described herein may have monomer units represented by the formula, in addition to the all regular 1,2-connection.



where j, k and m are each, independently, 1, 2, 3, 4, 5, 6, 7, 8, 9, 10, 11, 12, 13, 14, 15, 16, 17, 18, 19, 20, 21, or 22, n is an integer from 1 to 350 (preferably 1 to 300, preferably 5 to 50) as measured by proton NMR

In another embodiment, any of the polyalpha-olefins described herein preferably have an Mw (weight average molecular weight) of 100,000 or less, preferably between 100 and 80,000, preferably between 250 and 60,000, preferably between 280 and 50,000, preferably between 336 and 40,000 g/mol.

In another embodiment, any of the polyalpha-olefins described herein preferably have a Mn (number average molecular weight) of 50,000 or less, preferably between 200 and 40,000, preferably between 250 and 30,000, preferably between 500 and 20,000 g/mole.

## 12

In another embodiment, any of the polyalpha-olefins described herein preferably have a molecular weight distribution (MWD=Mw/Mn) of greater than 1 and less than 5, preferably less than 4, preferably less than 3, preferably less than 2.5. The MWD of mPAO is always a function of fluid viscosity. Alternately any of the polyalpha-olefins described herein preferably have an Mw/Mn of between 1 and 2.5, alternately between 1 and 3.5, depending on fluid viscosity.

The Mw, Mn and Mz are measured by GPC method using 10 a column for medium to low molecular weight polymers, tetrahydrofuran as solvent and polystyrene as calibration standard, correlated with the fluid viscosity according to a power equation.

In a preferred embodiment of this invention, any PAO 15 described herein may have a pour point of less than 0° C. (as measured by ASTM D 97), preferably less than -10° C., preferably less than -20° C., preferably less than -25° C., preferably less than -30° C., preferably less than -35° C., preferably less than -50°, preferably between -10 and -80° C., preferably between -15° C. and -70° C.

In a preferred embodiment of this invention, any PAO 20 described herein may have a kinematic viscosity (at 40° C. as measured by ASTM D 445) from about 4 to about 50,000 cSt, preferably from about 5 cSt to about 30,000 cSt at 40° C., alternately from about 4 to about 100,000 cSt, preferably from about 6 cSt to about 50,000 cSt, preferably from about 10 cSt to about 30,000 cSt at 40° C.

In another embodiment, any polyalpha-olefin described 25 herein may have a kinematic viscosity at 100° C. from about 1.5 to about 5,000 cSt, preferably from about 2 to about 3,000 cSt, preferably from about 3 cSt to about 1,000 cSt, more preferably from about 4 cSt to about 1,000 cSt, and yet more preferably from about 8 cSt to about 500 cSt as measured by ASTM D445. The PAOs preferably have viscosities in the range of 2 to 500 cSt at 100° C. in one embodiment, and from 2 to 3000 cSt at 100° C. in another embodiment, and from 3.2 to 300 cSt in another embodiment. Alternately, the polyalpha-olefin has a KV100 of less than 200 cSt.

In another embodiment, any polyalpha olefin described 30 herein may have a kinematic viscosity at 100° C. from 3 to 10 cSt and a flash point of 150° C. or more, preferably 200° C. or more (as measured by ASTM D 56).

In another embodiment, any polyalpha olefin described herein may have a dielectric constant of 2.5 or less (1 kHz at 45 23° C. as determined by ASTM D 924).

In another embodiment, any polyalpha olefin described herein may have a specific gravity of 0.75 to 0.96 g/cm<sup>3</sup>, preferably 0.80 to 0.94 g/cm<sup>3</sup>.

In another embodiment, any polyalpha olefin described 50 herein may have a viscosity index (VI) of 100 or more, preferably 120 or more, preferably 130 or more, alternately, from 120 to 450, alternately from 100 to 400, alternately from 120 to 380, alternately from 100 to 300, alternately from 140 to 380, alternately from 180 to 306, alternately from 252 to 306, 55 alternately the viscosity index is at least about 165, alternately at least about 187, alternately at least about 200, alternately at least about 252. For many lower viscosity fluids made from 1-decene or 1-decene equivalent feeds (KV100° C. of 3 to 10 cSt), the preferred VI range is from 100 to 180. Viscosity index is determined according to ASTM Method D 2270-93 [1998].

All kinematic viscosity values reported for fluids herein are measured at 100° C. unless otherwise noted. Dynamic viscosity can then be obtained by multiplying the measured 60 kinematic viscosity by the density of the liquid. The units for kinematic viscosity are in m<sup>2</sup>/s, commonly converted to cSt or centistokes (1 cSt=10<sup>-6</sup> m<sup>2</sup>/s or 1 cSt=1 mm<sup>2</sup>/sec).

One embodiment is a new class of poly-alpha-olefins, which have a unique chemical composition characterized by a high degree of linear branches and very regular structures with some unique head-to-head connections at the end position of the polymer chain. The polyalpha-olefins, whether homo-polymers or co-polymers, can be isotactic, syndiotactic or atactic polymers, or have combination of the tacticity. The new poly-alpha-olefins when used by themselves or blended with other fluids have unique lubrication properties.

Another embodiment is a new class of hydrogenated poly-alpha-olefins having a unique composition which is characterized by a high percentage of unique head-to-head connection at the end position of the polymer and by a reduced degree tacticity compared to the product before hydrogenation. The new poly-alpha-olefins when used by itself or blended with another fluid have unique lubrication properties.

This improved process to produce these polymers employs metallocene catalysts together with one or more activators (such as an alumoxane or a non-coordinating anion) and optionally with co-activators such as trialkylaluminum compounds. The metallocene catalyst can be a bridged or unbridged, substituted or unsubstituted cyclopentadienyl, indenyl or fluorenyl compound. One preferred class of catalysts are highly substituted metallocenes that give high catalyst productivity and higher product viscosity. Another preferred class of metallocenes are bridged and substituted cyclopentadienes. Another preferred class of metallocenes are bridged and substituted indenes or fluorenes. One aspect of the processes described herein also includes treatment of the feed olefins to remove catalyst poisons, such as peroxides, oxygen, sulfur, nitrogen-containing organic compounds, and/or acetylenic compounds. This treatment is believed to increase catalyst productivity, typically more than 5 fold, preferably more than 10 fold.

A preferred embodiment is a process to produce a polyalpha-olefin comprising:

1) contacting at least one alpha-olefin monomer having 3 to 30 carbon atoms with a metallocene compound and an activator under polymerization conditions wherein hydrogen, if present, is present at a partial pressure of 200 psi (1379 kPa) or less, based upon the total pressure of the reactor (preferably 150 psi (1034 kPa) or less, preferably 100 psi (690 kPa) or less, preferably 50 psi (345 kPa) or less, preferably 25 psi (173 kPa) or less, preferably 10 psi (69 kPa) or less (alternately the hydrogen, if present in the reactor at 30,000 ppm or less by weight, preferably 1,000 ppm or less preferably 750 ppm or less, preferably 500 ppm or less, preferably 250 ppm or less, preferably 100 ppm or less, preferably 50 ppm or less, preferably 25 ppm or less, preferably 10 ppm or less, preferably 5 ppm or less), and wherein the alpha-olefin monomer having 3 to 30 carbon atoms is present at 10 volume % or more based upon the total volume of the catalyst/activator/co-activator solutions, monomers, and any diluents or solvents present in the reaction; and

2) obtaining a polyalpha-olefin, optionally hydrogenating the PAO, and obtaining a PAO, comprising at least 50 mole % of a C3 to C30 alpha-olefin monomer, wherein the polyalpha-olefin has a kinematic viscosity at 100° C. of 5000 cSt or less, and the polyalpha-olefin comprises Z mole % or more of units represented by the formula:



where j, k and m are each, independently, 1, 2, 3, 4, 5, 6, 7, 8, 9, 10, 11, 12, 13, 14, 15, 16, 17, 18, 19, 20, 21, or 22, n is an integer from 1 to 350, and

An alternate embodiment is a process to produce a polyalpha-olefin comprising:

1) contacting a feed stream comprising one or at least one alpha-olefin monomer having 3 to 30 carbon atoms with a metallocene catalyst compound and a non-coordinating anion activator or alkylalumoxane activator, and optionally an alkyl-aluminum compound, under polymerization conditions wherein the alpha-olefin monomer having 3 to 30 carbon atoms is present at 10 volume % or more based upon the total volume of the catalyst/activator/co-activator solution, monomers, and any diluents or solvents present in the reactor and where the feed alpha-olefin, diluent or solvent stream comprises less than 300 ppm of heteroatom containing compounds; and obtaining a polyalpha-olefin comprising at least 50 mole % of a C5 to C24 alpha-olefin monomer where the polyalpha-olefin has a kinematic viscosity at 100° C. of 5000 cSt or less. Preferably, hydrogen, if present is present in the reactor at 30,000 ppm or less by weight, preferably 1,000 ppm or less preferably 750 ppm or less, preferably 500 ppm or less, preferably 250 ppm or less, preferably 100 ppm or less, preferably 50 ppm or less, preferably 25 ppm or less, preferably 10 ppm or less, preferably 5 ppm or less.

An alternate embodiment is a process to produce a polyalpha-olefin comprising:

1) contacting a feed stream comprising at least one alpha-olefin monomer having 3 to 30 carbon atoms with a metallocene catalyst compound and a non-coordinating anion activator or alkylalumoxane activator, and optionally an alkyl-aluminum compound, under polymerization conditions wherein the alpha-olefin monomer having 3 to 30 carbon atoms is present at 10 volume % or more based upon the total volume of the catalyst/activator/co-activator solution, monomers, and any diluents or solvents present in the reactor and where the feed alpha-olefin, diluent or solvent stream comprises less than 300 ppm of heteroatom containing compounds; and obtaining a polyalpha-olefin comprising at least 50 mole % of a C5 to C24alpha-olefin monomer where the polyalpha-olefin has a kinematic viscosity at 100° C. of 5000 cSt or less; Alternately, in this process described herein hydrogen, if present, is present in the reactor at 1000 ppm or less by weight, preferably 750 ppm or less, preferably 500 ppm or less, preferably 250 ppm or less, preferably 100 ppm or less, preferably 50 ppm or less, preferably 25 ppm or less, preferably 10 ppm or less, preferably 5 ppm or less.

2) isolating the lube fraction polymers and then contacting this lube fraction with hydrogen under typical hydrogenation conditions with hydrogenation catalyst to give fluid with bromine number below 1.8, or alternatively, isolating the lube fraction polymers and then contacting this lube fraction with hydrogen under more severe conditions with hydrogenation catalyst to give fluid with bromine number below 1.8 and with reduce mole % of mm components than the unhydrogenated polymers. The hydrogen pressure for this process is usually in the range from 50 psi to 3000 psi, preferably 200 to 2000 psi, preferably 500 to 1500 psi.

#### Molecular Weight Distribution (MWD)

Molecular weight distribution is a function of viscosity. The higher the viscosity the higher the molecular weight distribution. FIG. 1 is a graph showing the molecular weight distribution as a function of viscosity at Kv100° C. The circles represent the prior art prior PAO. The squares and upper triangles represent the new metallocene catalyzed PAOs. Line 1 represents the preferred lower range of molecular weight distribution for the high viscosity metallocene catalyzed PAO. Line 3 represents preferred upper range of the molecular weight distribution for the high viscosity metallocene catalyzed PAO. Therefore, the region bounded by lines 1 and

3 represents the preferred molecular weight distribution region of the new metallocene catalyzed PAO. Line 2 represents the desirable and typical MWD of actual experimental samples of the metallocene PAO made from 1-decene. Line 5 represents molecular weight distribution of the prior art PAO.

Equation 1 represents the algorithm for line 5 or the average molecular weight distribution of the prior art PAO. Whereas equations 2, 3, and 4 represent lines 1, 3 and 2 respectively.

$$\text{MWD} = 0.2223 + 1.0232 * \log(\text{Kv at } 100^\circ \text{ C. in cSt}) \quad \text{Eq. 1}$$

$$\text{MWD} = 0.41667 + 0.725 * \log(\text{Kv at } 100^\circ \text{ C. in cSt}) \quad \text{Eq. 2}$$

$$\text{MWD} = 0.8 + 0.3 * \log(\text{Kv at } 100^\circ \text{ C. in cSt}) \quad \text{Eq. 3}$$

$$\text{MWD} = 0.66017 + 0.44922 * \log(\text{Kv at } 100^\circ \text{ C. in cSt}) \quad \text{Eq. 4}$$

In at least one embodiment, the molecular weight distribution is at least 10 percent less than equation 1. In a preferred embodiment the molecular weight distribution is less than equation 2 and in a most preferred embodiment the molecular weight distribution is less than equation 2 and more than equation 4.

Table 3 is a table demonstrating the differences between metallocene catalyzed PAO ("mPAO") and current high viscosity prior art PAO (cHVI-PAO). Examples 1 to 8 in the Table 1 were prepared from different feed olefins using metallocene catalysts. The metallocene catalyst system, products, process and feeds were described in Patent Applications Nos. PCT/US2006/021399 and PCT/US2006/021231. The mPAOs samples in Table were made from C10, C6,12, C6 to C18, C6,10,14-LAOs. Examples 1 to 7 samples all have very narrow molecular weight distribution (MWD). The MWD of mPAO depends on fluid viscosity as shown in FIG. 1.

U.S. Pat. Nos. 4,827,064 and 4,827,073. They have broad MWD and therefore poor shear stability in TRB test.

The comparison of shear stability as a function of fluid viscosity for mPAO with narrow MWD vs. cHVI-PAO is summarized in FIG. 2. This graph demonstrates that the mPAO profile shown as line 21 has much improved shear stability over wide viscosity range when compared to the cHVI-PAO profile shown as line 23.

These examples demonstrated the importance of MWD effect on shear stability. Accordingly, The higher viscosity base stocks with tighter molecular weight distributions provide favorable shear stability even at high viscosities.

#### Lubricant Formulation

The formulation is based on extreme modal blends of high viscosity synthetic group IV PAO. In a preferred embodiment, a High Viscosity Index, metallocene-catalyzed PAO of greater than 100 cSt is blended with a low-viscosity base stock PAO and/or with one or more of Gr V base stocks, such as an ester, a polyalkylene glycol or an alkylated aromatic, as a co-base for additive solubility. A detailed description of suitable Gr V base stocks can be found in "Synthetics, Mineral Oils and Bio-Based Lubricants, Chemistry and Technology" Edited by L. R. Rudnick, published by CRC Press, Taylor & Francis, 2005. The esters of choice are dibasic esters (such as adipate ester, ditridecyl adipate), mono-basic esters, polyol esters and phthalate esters. The alkylated aromatics of choice are alkylbenzene, alkylated naphthalene and other alkylated aromatics such as alkylated diphenylether, diphenylsulfide, biphenyl, etc. We have found that this unique base stock combination can impart enhanced worm gear efficiency, improved air-release property and decrease in operating temperature.

TABLE 5

| sample type                | Example No. |        |        |          |          |        |         |          |          |          |        |
|----------------------------|-------------|--------|--------|----------|----------|--------|---------|----------|----------|----------|--------|
|                            | 1           | 2      | 3      | 4        | 5        | 6      | 7       | 8        | 9        | 10       | 11     |
| mPAO                       | mPAO        | mPAO   | mPAO   | mPAO     | mPAO     | mPAO   | mPAO    | cHVI-PAO | cHVI-PAO | cHVI-PAO |        |
| C6/C12                     | C6-C18      | C6-C18 | C10    | C6,10,14 | C6,10,14 | C10    | C10     | C10      | C10      | C10      |        |
| 100° C. Kv, cS             | 150         | 151    | 540    | 671      | 460      | 794.35 | 1386.63 | 678.1    | 150      | 300      | 1,000  |
| 40° C. Kv, cS              | 1701        | 1600   | 6642   | 6900     | 5640     | 10318  | 16362   | 6743     | 1500     | 3100     | 10,000 |
| VI                         | 199         | 207    | 257    | 248      | 275      | 321    | 303     | 218      | 241      | 307      |        |
| Pour. ° C.                 | -33         | -36    | -21    | -18      | nd       | nd     | -12     | -33      | -27      | -18      |        |
| MWD by GPC                 |             |        |        |          |          |        |         |          |          |          |        |
| Mw                         | 7,409       | 8,089  | 17,227 | 19,772   | 16,149   | 20,273 | 31,769  | 29,333   | 8,974    | 12,511   | 32,200 |
| MWD                        | 1.79        | 2.01   | 1.90   | 1.98     | 2.35     | 2.18   | 1.914   | 5.50     | 2.39     | 2.54     | 4.79   |
| % Visc Change TRB Test (a) |             |        |        |          |          |        |         |          |          |          |        |
| 20 hrs                     | -0.33       | -0.65  | -2.66  | -3.64    | -4.03    | -8.05  | -19.32  | -29.11   | -7.42    | -18.70   | -46.78 |
| 100 hrs                    | -0.83       | -0.70  | -1.07  | 1.79     | nd       | nd     | nd      | nd       | nd       | -21.83   | -51.09 |

(a) CEC L-45-A-99 Taper Roller Bearing/C (20 hours) (KRL test 20 hours) at SouthWest Research Institute

When Example 1 to 7 samples were subjected to tapered roller bearing ("TRB") test, they show very low viscosity loss after 20 hours shearing or after extended 100 hours shearing (TRB). Generally, shear stability is a function of fluid viscosity. Lower viscosity fluids have minimal viscosity losses of less than 10%. When fluid viscosity is above 1000 cSt as in Example 7, the fluid loss is approximately 19% viscosity. Example 8 is a metallocene PAO with MWD of 5.5. This metallocene PAO shows significant amount of viscosity loss at 29%.

Examples 9, 10 and 11 are comparative examples. The high viscosity PAO are made according to methods described in

Also, unexpected and significant air release benefits result from this discovery. Specifically, decreased air release times according to ASTM D 3427. These air release benefits are manifest in a decrease of as much as 75% of the standard release times of gear oil viscosity-grade lubricants. In addition to the above mentioned benefits, we also discovered, significant improvements in low temperature performance (reduction in pour point).

In one embodiment, the lubricant oil comprises at least two base stock blends of oil. The first base stock blend comprises lubricant oil with a viscosity of over 300 cSt, and more preferably over 400 cSt, Kv100° C. Most preferably, the base stock is over 570 cSt, Kv100° C. but less than 5000 cSt. The

first base stock has a molecular weight distribution less than 10 percent of equation 1. In an even more preferred embodiment the first base stock is a metallocene catalyzed PAO with a viscosity of at least 300, more preferably 400 and most preferably at least 600 cSt.

The second base stock blend comprises a lubricant oil with a viscosity of less than 60 cSt and preferably less than 40 cSt, and most preferably less than 10 cSt. Preferably, the viscosity of the second lubricant should be at least 1.5 cSt. Even more preferable is a viscosity of between 1.7 and 40 cSt.

The air release performance enhancement of the current invention is an unexpected result since the typical performance of these very viscous oils (ISO 460) is typically an air release time to 0.2% air in the ASTM D3427 test to be 20 minutes or more. Also, the low temperature performance of these preferred base stock shows significant improvement as demonstrated in the ASTM D97 and D5133 data shown in Table 4. The air release performance enhancement of these base stock combinations are important since the typical performance of these very viscous oils (ISO 460) is typically an air release time to 0.2% air in the ASTM D3427 test to be 20 minutes or more.

TABLE 6

| Air Release<br>in Minutes | ASTM D3427 (75 C.)                             |                                               | Commercially<br>available ISO 460<br>Gear Oil |
|---------------------------|------------------------------------------------|-----------------------------------------------|-----------------------------------------------|
|                           | Results<br>Bi-model PAO ISO<br>460<br>Gear Oil | Commercially<br>available ISO 460<br>Gear Oil |                                               |
| Time to 0.1% air          | 6.9                                            | 25                                            |                                               |
| Time to 0.2% air          | 5.2                                            | 21                                            |                                               |

Groups I, II, III, IV and V are broad categories of base oil stocks developed and defined by the American Petroleum Institute (API Publication 1509; [www.API.org](http://www.API.org)) to create guidelines for lubricant base oils. Group I base stocks generally have a viscosity index of between about 80 to 120 and contain greater than about 0.03% sulfur and/or less than about 90% saturates. Group II base stocks generally have a viscosity index of between about 80 to 120, and contain less than or equal to about 0.03% sulfur and greater than or equal to about 90% saturates. Group III stock generally has a viscosity index greater than about 120 and contains less than or equal to about 0.03% sulfur and greater than about 90% saturates. Group IV includes polyalphaolefins (PAO). Group V base stocks include base stocks not included in Groups I-IV. Table 5 summarizes properties of each of these five groups. All discussion of Gr I to V base stocks can be found in "Synthetics, Mineral Oils and Bio-Based Lubricants, Chemistry and Technology" Edited by L. R. Rudnick, published by CRC Press, Taylor & Francis, 2005.

Group VI in Table 5 are Polyinternal olefins ("PIO"). Polyinternal olefins are long-chain hydrocarbons, typically a linear backbone with some branching randomly attached; they are obtained by oligomerization of internal n-olefins. The catalyst is usually a BF<sub>3</sub> complex with a proton source that leads to a cationic polymerization, or promoted BF<sub>3</sub> or AlCl<sub>3</sub> catalyst system. The process to produce polyinternal olefins (PIO) consists of four steps: reaction, neutralization/washing, hydrogenation and distillation. These steps are somewhat similar to PAO process. PIO are typically available in low viscosity grades, 4 cS, 6 cS and 8 cS. If necessary, low viscosity, 1.5 to 3.9 cS can also be made conveniently by the BF<sub>3</sub> process or other cationic processes. Typically, the n-olefins used as starting material are n-C<sub>12</sub>-C<sub>18</sub> internal olefins, more preferably, n-C<sub>14</sub>-C<sub>16</sub> olefins are used. PIO can be

made with VI and pour points very similar to PAO, only slightly inferior. They can be used in engine and industrial lubricant formulations. For more detailed discussion, see Chapter 2, Polyinternalolefins in the book, "Synthetics, Mineral Oils, and Bio-Based Lubricants—Chemistry and Technology" Edited by Leslie R. Rudnick, p. 37-46, published by CRC Press, Taylor & Francis Group, 2006; or "Polyinternal Olefins" by Corsico, G.; Mattei, L.; Roselli, A.; Gommellini, Carlo. EURON. Milan, Italy. Chemical Industries (Dekker) 10 (1999), 77(Synthetic Lubricants and High-Performance Functional Fluids, (2nd Edition)), 53-62. Publisher: Marcel Dekker, Inc. PIO was classified by itself as Group IV fluid in API base stock classification.

TABLE 7

| Base Stock Properties |             |                                                                       |                 |
|-----------------------|-------------|-----------------------------------------------------------------------|-----------------|
|                       | Saturates   | Sulfur                                                                | Viscosity Index |
| Group I               | <90% and/or | >0.03% and                                                            | ≥80 and <120    |
| Group II              | ≥90% and    | ≤0.03% and                                                            | ≥80 and <120    |
| Group III             | ≥90% and    | ≤0.03% and                                                            | ≥120            |
| Group IV              |             | Polyalphaolefins (PAO)                                                |                 |
| Group V               |             | All other base oil stocks not included<br>in Groups I, II, III, or IV |                 |
| Group VI              |             | Polyinternal olefins (PIO)                                            |                 |

In a preferred embodiment, the base stocks include at least one base stock of synthetic oils and most preferably include at least one base stock of API group IV Poly Alpha Olefins. Synthetic oil for purposes of this application shall include all oils that are not naturally occurring mineral oils. Naturally occurring mineral oils are often referred to as API Group I oils.

A new type of PAO lubricant was introduced by U.S. Pat. 35 Nos. 4,827,064 and 4,827,073 (Wu). These PAO materials, which are produced by the use of a reduced valence state chromium catalyst, are olefin oligomers or polymers which are characterized by very high viscosity indices which give them very desirable properties to be useful as lubricant base stocks and, with higher viscosity grades; as VI improvers. 40 They are referred to as High Viscosity Index PAOs or HVI-PAOs. The relatively low molecular weight high viscosity PAO materials were found to be useful as lubricant base stocks whereas the higher viscosity PAOs, typically with 45 viscosities of 100 cSt or more, e.g. in the range of 100 to 1,000 cSt, were found to be very effective as viscosity index improvers for conventional PAOs and other synthetic and mineral oil derived base stocks.

Various modifications and variations of these high viscosity PAO materials are also described in the following U.S. 50 patents to which reference is made: U.S. Pat. Nos. 4,990,709; 5,254,274; 5,132,478; 4,912,272; 5,264,642; 5,243,114; 5,208,403; 5,057,235; 5,104,579; 4,943,383; 4,906,799. These oligomers can be briefly summarized as being produced by the oligomerization of 1-olefins in the presence of a 55 metal oligomerization catalyst which is a supported metal in a reduced valence state. The preferred catalyst comprises a reduced valence state chromium on a silica support, prepared by the reduction of chromium using carbon monoxide as the reducing agent. The oligomerization is carried out at a temperature selected according to the viscosity desired for the 60 resulting oligomer, as described in U.S. Pat. Nos. 4,827,064 and 4,827,073. Higher viscosity materials may be produced as described in U.S. Pat. No. 5,012,020 and U.S. Pat. No. 65 5,146,021 where oligomerization temperatures below about 90° C. are used to produce the higher molecular weight oligomers. In all cases, the oligomers, after hydrogenation when

necessary to reduce residual unsaturation, have a branching index (as defined in U.S. Pat. Nos. 4,827,064 and 4,827,073) of less than 0.19. Overall, the HVI-PAO normally have a viscosity in the range of about 12 to 5,000 cSt.

Furthermore, the HVI-PAOs generally can be characterized by one or more of the following: C30-C1300 hydrocarbons having a branch ratio of less than 0.19, a weight average molecular weight of between 300 and 45,000, a number average molecular weight of between 300 and 18,000, a molecular weight distribution of between 1 and 5. Particularly preferred HVI-PAOs are fluids with 100° C. viscosity ranging from 5 to 5000 cSt. In another embodiment, viscosities of the HVI-PAO oligomers measured at 100° C. range from 3 centistokes ("cSt") to 15,000 cSt. Furthermore, the fluids with viscosity at 100° C. of 3 cSt to 5000 cSt have VI calculated by ASTM method D2270 greater than 130. Usually they range from 130 to 350. The fluids all have low pour points, below -15° C.

The HVI-PAOs can further be characterized as hydrocarbon compositions comprising the polymers or oligomers made from 1-alkenes, either by itself or in a mixture form, taken from the group consisting of C6-C20 1-alkenes. Examples of the feeds can be 1-hexene, 1-octene, 1-decene, 1-dodecene, 1-tetradecene, etc. or mixture of C6 to C14 1-alkenes or mixture of C6 to C20 1-alkenes, C6 and C12 1-alkenes, C6 and C14 1-alkenes, C6 and C16 1-alkenes, C6 and C18 1-alkenes, C8 and C10 1-alkenes, C8 and C12 1-alkenes, C8, C10 and C12 1-alkenes, and other appropriate combinations.

The lube products usually are distilled to remove any low molecular weight compositions such as these boiling below 600° F., or with carbon number less than C20, if they are produced from the polymerization reaction or are carried over from the starting material. This distillation step usually improves the volatility of the finished fluids. In certain special applications, or when no low boiling fraction is present in the reaction mixture, this distillation is not necessary. Thus the whole reaction product after removing any solvent or starting material can be used as lube base stock or for the further treatments.

The lube fluids made directly from the polymerization or oligomerization process usually have unsaturated double bonds or have olefinic molecular structure. The amount of double bonds or unsaturation or olefinic components can be measured by several methods, such as bromine number (ASTM 1159), bromine index (ASTM D2710) or other suitable analytical methods, such as NMR, IR, etc. The amount of the double bond or the amount of olefinic compositions depends on several factors—the degree of polymerization, the amount of hydrogen present during the polymerization process and the amount of other promoters which participate in the termination steps of the polymerization process, or other agents present in the process. Usually, the amount of double bonds or the amount of olefinic components is decreased by the higher degree of polymerization, the higher amount of hydrogen gas present in the polymerization process, or the higher amount of promoters participating in the termination steps.

It was known that, usually, the oxidative stability and light or UV stability of fluids improves when the amount of unsaturation double bonds or olefinic contents is reduced. Therefore it is necessary to further hydrotreat the polymer if they have high degree of unsaturation. Usually, the fluids with bromine number of less than 5, as measured by ASTM D1159, is suitable for high quality base stock application. Of course, the lower the bromine number, the better the lube quality. Fluids with bromine number of less than 3 or 2 are

common. The most preferred range is less than 1 or less than 0.1. The method to hydrotreat to reduce the degree of unsaturation is well known in literature [U.S. Pat. No. 4,827,073, example 16]. In some HVI-PAO products, the fluids made directly from the polymerization already have very low degree of unsaturation, such as those with viscosities greater than 150 cSt at 100° C. They have bromine numbers less than 5 or even below 2. In these cases, we can chose to use as is without hydrotreating, or we can choose to hydrotreating to further improve the base stock properties.

Another type of PAO, classified as Group IV base stock and used extensively in many synthetic or partial synthetic industrial lubricants, is produced by oligomerization or polymerization of linear alpha-olefins of C6 to C16 by promoted BF3 or AlCl3 catalysts. This type of PAO is available in many viscosity grades ranging from 1.7 cS to 100 cS from Exxon-Mobil Chemical Co.

Base stocks having a high paraffinic/naphthenic and saturation nature of greater than 90 weight percent can often be used advantageously in certain embodiments. Such base stocks include Group II and/or Group III hydroprocessed or hydrocracked base stocks, or their synthetic counterparts such as polyalphaolefin oils, GTL or similar base oils or mixtures of similar base oils. For purposes of this application synthetic bases stocks shall include Group II, Group III, group IV and Group V base stocks.

A more specific example embodiment, is the combination of high viscosity metallocene catalyzed PAO having a molecular weight distribution (MWD) as a function of viscosity at least 10 percent less than the algorithm: [MWD=0.2223+1.0232\*log (Kv at 100° C. in cSt)] with a low viscosity Poly Alpha Olefin ("PAO") including PAOs with a viscosity of less than 6 cSt, and more preferably with a viscosity between 1.5 cSt or 4 cSt, Kv100° C. and even more preferably with a small amount of Group V base stocks, including esters, polyalkylene glycols, or alkylated aromatics. The Gr V base stocks can be used as an additional base stock or as a co-base stock with either the first and second base stocks for additive solubility. The preferred ester is an alkyl adipate, a polyol ester or aromatic ester, such as phthalate ester. The preferred alkyl aromatics are alkylbenzenes or alkylnaphthalenes. The preferred polyalkylene glycols are liquid polymers or copolymers made from ethylene oxide, propylene oxide, butylenes oxides or higher alkylene oxides with some degree of compatibility with PAO, other hydrocarbon fluids, GTL or mineral oils.

Gas to liquid (GTL) base stocks can also be preferentially used with the components of this invention as a portion or all of the base stocks used to formulate the finished lubricant. We have discovered, favorable improvement when the components of this invention are added to lubricating systems comprising primarily Group II, Group III and/or GTL base stocks compared to lesser quantities of alternate fluids.

GTL materials are materials that are derived via one or more synthesis, combination, transformation, rearrangement, and/or degradation/deconstructive processes from gaseous carbon-containing compounds, hydrogen-containing compounds, and/or elements as feedstocks such as hydrogen, carbon dioxide, carbon monoxide, water, methane, ethane, ethylene, acetylene, propane, propylene, propyne, butane, butylenes, and butynes. GTL base stocks and base oils are GTL materials of lubricating viscosity that are generally derived from hydrocarbons, for example waxy synthesized hydrocarbons, that are themselves derived from simpler gaseous carbon-containing compounds, hydrogen-containing compounds and/or elements as feedstocks. GTL base stock(s) include oils boiling in the lube oil boiling range separated/

fractionated from GTL materials such as by, for example, distillation or thermal diffusion, and subsequently subjected to well-known catalytic or solvent dewaxing processes to produce lube oils of reduced/low pour point; wax isomerates, comprising, for example, hydroisomerized or isodewaxed synthesized hydrocarbons; hydro-isomerized or isodewaxed Fischer-Tropsch ("F-T") material (i.e., hydrocarbons, waxy hydrocarbons, waxes and possible analogous oxygenates); preferably hydroisomerized or isodewaxed F-T hydrocarbons or hydroisomerized or isodewaxed F-T waxes, hydroisomerized or isodewaxed synthesized waxes, or mixtures thereof.

GTL base stock(s) derived from GTL materials, especially, hydroisomerized/isodewaxed F-T material derived base stock(s), and other hydroisomerized/isodewaxed wax derived base stock(s) are characterized typically as having kinematic viscosities at 100° C. of from about 2 mm<sup>2</sup>/s to about 50 mm<sup>2</sup>/s, preferably from about 3 mm<sup>2</sup>/s to about 50 mm<sup>2</sup>/s, more preferably from about 3.5 mm<sup>2</sup>/s to about 30 mm<sup>2</sup>/s, as exemplified by a GTL base stock derived by the isodewaxing of F-T wax, which has a kinematic viscosity of about 4 mm<sup>2</sup>/s at 100° C. and a viscosity index of about 130 or greater. The term GTL base oil/base stock and/or wax isomerate base oil/base stock as used herein and in the claims is to be understood as embracing individual fractions of GTL base stock/base oil or wax isomerate base stock/base oil as recovered in the production process, mixtures of two or more GTL base stocks/base oil fractions and/or wax isomerate base stocks/base oil fractions, as well as mixtures of one or two or more low viscosity GTL base stock(s)/base oil fraction(s) and/or wax isomerate base stock(s)/base oil fraction(s) with one, two or more high viscosity GTL base stock(s)/base oil fraction(s) and/or wax isomerate base stock(s)/base oil fraction(s) to produce a bi-modal blend wherein the blend exhibits a viscosity within the aforesaid recited range. Reference herein to Kinematic Viscosity refers to a measurement made by ASTM method D445.

GTL base stocks and base oils derived from GTL materials, especially hydroisomerized/isodewaxed F-T material derived base stock(s), and other hydroisomerized/isodewaxed wax-derived base stock(s), such as wax hydroisomerates/isodewaxates, which can be used as base stock components of this invention are further characterized typically as having pour points of about -5° C. or lower, preferably about -10° C. or lower, more preferably about -15° C. or lower, still more preferably about -20° C. or lower, and under some conditions may have advantageous pour points of about -25° C. or lower, with useful pour points of about -30° C. to about -40° C. or lower. If necessary, a separate dewaxing step may be practiced to achieve the desired pour point. References herein to pour point refer to measurement made by ASTM D97 and similar automated versions.

The GTL base stock(s) derived from GTL materials, especially hydroisomerized/isodewaxed F-T material derived base stock(s), and other hydroisomerized/isodewaxed wax-derived base stock(s) which are base stock components which can be used in this invention are also characterized typically as having viscosity indices of 80 or greater, preferably 100 or greater, and more preferably 120 or greater. Additionally, in certain particular instances, viscosity index of these base stocks may be preferably 130 or greater, more preferably 135 or greater, and even more preferably 140 or greater. For example, GTL base stock(s) that derive from GTL materials preferably F-T materials especially F-T wax generally have a viscosity index of 130 or greater. References herein to viscosity index refer to ASTM method D2270.

In addition, the GTL base stock(s) are typically highly paraffinic of greater than 90 percent saturates) and may contain mixtures of monocycloparaffins and multicycloparaffins in combination with non-cyclic isoparaffins. The ratio of the 5 naphthenic (i.e., cycloparaffin) content in such combinations varies with the catalyst and temperature used. Further, GTL base stocks and base oils typically have very low sulfur and nitrogen content, generally containing less than about 10 ppm, and more typically less than about 5 ppm of each of 10 these elements. The sulfur and nitrogen content of GTL base stock and base oil obtained by the hydroisomerization/isodewaxing of F-T material, especially F-T wax is essentially nil.

In a preferred embodiment, the GTL base stock(s) comprises paraffinic materials that consist predominantly of non-cyclic isoparaffins and only minor amounts of cycloparaffins. 15 These GTL base stock(s) typically comprise paraffinic materials that consist of greater than 60 wt % non-cyclic isoparaffins, preferably greater than 80 wt % non-cyclic isoparaffins, more preferably greater than 85 wt % non-cyclic isoparaffins, and most preferably greater than 90 wt % non-cyclic isoparaffins.

Useful compositions of GTL base stock(s), hydroisomerized or isodewaxed F-T material derived base stock(s), and wax-derived hydroisomerized/isodewaxed base stock(s), 25 such as wax isomerates/isodewaxates, are recited in U.S. Pat. Nos. 6,080,301; 6,090,989, and 6,165,949 for example. Additives

We have discovered that this unique base stock combination can impart even further favorable properties when combined with the specific novel additive system disclosed 30 herein. The additives include various commercially available gear oil packages. These additive packages include a high performance series of components that include antiwear, antioxidant, defoamant, demulsifier, detergent, dispersant, metal 35 passivation, and rust inhibition additive chemistries to deliver desired performance.

The additives may be chosen to modify various properties of the lubricating oils. For gear oils, the additives should provide the following properties, antiwear protection, rust 40 protection, micropitting protection, friction reduction, and improved filterability. Persons skilled in the art based on the disclosure herein will recognize various additive combinations that can be chosen to achieve favorable properties including favorable properties for gear oil applications.

In a high viscosity embodiment, the final lubricant should comprise a first lubricant base stock having a viscosity of greater than 100 cSt, Kv100° C. The first lubricant base stock should comprise of at least 10 percent and no more than 70 percent of the final lubricant. Preferred range is at least 20 percent to 60 percent. The second base stock having a viscosity less than 100 cSt should comprise at least 20 percent and no more than 70 percent of the final base stock total. The amount of Group V base stocks, such as esters, polyalkylene glycols or alkylated aromatics and/or additive can be up to 90 percent of the final lubricant total with a proportional decrease in the acceptable ranges of first and second base stocks. The preferred range of group V, such as esters and additives is between 10 and 90 percent. Sometimes, some Group I or II base stock can be used in the formulation 55 together with ester or alkylated aromatics or as a total substitute.

In various embodiments, it will be understood that additives well known as functional fluid additives in the art, can also be incorporated in the functional fluid composition of the 60 invention, in relatively small amounts, if desired; frequently, less than about 0.001% up to about 10-20% or more. In one embodiment, at least one oil additive is added from the group

consisting of antioxidants, stabilizers, antiwear additives, dispersants, detergents, anti foam additives, viscosity index improvers, copper passivators, metal deactivators, rust inhibitors, corrosion inhibitors, pour point depressants, demulsifiers, anti-wear agents, extreme pressure additives and friction modifiers. The additives listed below are non-limiting examples and are not intended to limit the claims.

Dispersants should contain the alkenyl or alkyl group R has an Mn value of about 500 to about 5000 and an Mw/Mn ratio of about 1 to about 5. The preferred Mn intervals depend on the chemical nature of the agent improving filterability. Polyolefinic polymers suitable for the reaction with maleic anhydride or other acid materials or acid forming materials, include polymers containing a predominant quantity of C2 to C5 monoolefins, for example ethylene, propylene, butylene, isobutylene and pentene. A highly suitable polyolefinic polymer is polyisobutene. The succinic anhydride preferred as a reaction substance is PIBSA, that is, polyisobutylene succinic anhydride.

If the dispersant contains a succinimide comprising the reaction product of a succinic anhydride with a polyamine, the alkenyl or alkyl substituent of the succinic anhydride serving as the reaction substance consists preferably of polymerised isobutene having an Mn value of about 1200 to about 2500. More advantageously, the alkenyl or alkyl substituent of the succinic anhydride serving as the reaction substance consists in a polymerised isobutene having an Mn value of about 2100 to about 2400. If the agent improving filterability contains an ester of succinic acid comprising the reaction product of a succinic anhydride and an aliphatic polyhydric alcohol, the alkenyl or alkyl substituent of the succinic anhydride serving as the reaction substance consists advantageously of a polymerised isobutene having an Mn value of 500 to 1500. In preference, a polymerised isobutene having an Mn value of 850 to 1200 is used.

Amides suitable uses of amines include antiwear agents, extreme pressure additives, friction modifiers or Dispersants. The amides which are utilized in the compositions of the present invention may be amides of mono- or polycarboxylic acids or reactive derivatives thereof. The amides may be characterized by a hydrocarbyl group containing from about 6 to about 90 carbon atoms; each is independently hydrogen or a hydrocarbyl, aminohydrocarbyl, hydroxyhydrocarbyl or a heterocyclic-substituted hydrocarbyl group, provided that both are not hydrogen; each is, independently, a hydrocarbylene group containing up to about 10 carbon atoms; Alk is an alkylenes group containing up to about 10 carbon atoms.

The amide can be derived from a monocarboxylic acid, a hydrocarbyl group containing from 6 to about 30 or 38 carbon atoms and more often will be a hydrocarbyl group derived from a fatty acid containing from 12 to about 24 carbon atoms.

The amide is derived from a di- or tricarboxylic acid, will contain from 6 to about 90 or more carbon atoms depending on the type of polycarboxylic acid. For example, when the amide is derived from a dimer acid, will contain from about 18 to about 44 carbon atoms or more, and amides derived from trimer acids generally will contain an average of from about 44 to about 90 carbon atoms. Each is independently hydrogen or a hydrocarbyl, aminohydrocarbyl, hydroxyhydrocarbyl or a heterocyclic-substituted hydrocarbon group containing up to about 10 carbon atoms. It may be independently heterocyclic substituted hydrocarbyl groups wherein the heterocyclic substituent is derived from pyrrole, pyrrolidine, pyrrolidine, morpholine, piperazine, piperidine, pyridine, pipecoline, etc. Specific examples include methyl, ethyl, n-propyl, n-butyl, n-hexyl, hydroxymethyl, hydroxy-

ethyl, hydroxypropyl, amino-methyl, aminoethyl, aminopropyl, 2-ethylpyridine, 1-ethylpyrrolidine, 1-ethylpiperidine, etc.

The alkyl group can be an alkylenes group containing from 5 to about 10 carbon atoms. Examples of such alkylenes groups include, methylene, ethylene, propylene, etc. Also are hydrocarbylene groups, and in particular, alkylenes group containing up to about 10 carbon atoms. Examples of such hydrocarbylene groups include, methylene, ethylene, propylene, etc. The amide contains at least one morpholinyl group. In one embodiment, the morpholine structure is formed as a result of the condensation of two hydroxy groups which are attached to the hydrocarbylene groups. Typically, the amides are prepared by reacting a carboxylic acid or reactive derivative thereof with an amine which contains at least one >NH group.

Aliphatic monoamines include mono-aliphatic and di-aliphatic-substituted amines wherein the aliphatic groups may be saturated or unsaturated and straight chain or branched chain. Such amines include, for example, mono- and di-alkyl-substituted amines, mono- and dialkenyl-substituted amines, etc. Specific examples of such monoamines include ethyl amine, diethyl amine, n-butyl amine, di-n-butyl amine, isobutyl amine, coco amine, stearyl amine, oleyl amine, etc. An example of a cycloaliphatic-substituted aliphatic amine is 2-(cyclohexyl)-ethyl amine. Examples of heterocyclic-substituted aliphatic amines include 2-(2-aminoethyl)-pyrrole, 2-(2-aminoethyl)-1-methyl pyrrole, 2-(2-aminoethyl)-1-methylpyrrolidine and 4-(2-aminoethyl)morpholine, 1-(2-aminoethyl)piperazine, 1-(2-aminoethyl)piperidine, 2-(2-aminoethyl)pyridine, 1-(2-aminoethyl)pyrrolidine, 1-(3-aminopropyl)imidazole, 3-(2-aminopropyl)indole, 4-(3-aminopropyl)morpholine, 1-(3-aminopropyl)-2-pipecoline, 1-(3-aminopropyl)-2-pyrrolidinone, etc.

Cycloaliphatic monoamines are those monoamines wherein there is one cycloaliphatic substituent attached directly to the amino nitrogen through a carbon atom in the cyclic ring structure. Examples of cycloaliphatic monoamines include cyclohexylamines, cyclopentylamines, cyclohexylamines, cyclopentenylamines, N-ethyl-cyclohexylamine, dicyclohexylamines, and the like. Examples of aliphatic-substituted, aromatic-substituted, and heterocyclic-substituted cycloaliphatic monoamines include propyl-substituted cyclohexyl-amines, phenyl-substituted cyclopentylamines, and pyranyl-substituted cyclohexylamine.

Aromatic amines include those monoamines wherein a carbon atom of the aromatic ring structure is attached directly to the amino nitrogen. The aromatic ring will usually be a mononuclear aromatic ring (i.e., one derived from benzene) but can include fused aromatic rings, especially those derived from naphthalene. Examples of aromatic monoamines include aniline, di-(para-methylphenyl)amine, naphthylamine, N-(n-butyl)-aniline, and the like. Examples of aliphatic-substituted, cycloaliphatic-substituted, and heterocyclic-substituted aromatic monoamines are para-ethoxyaniline, para-dodecylaniline, cyclohexyl-substituted naphthylamine, phenothiazines, and thienyl-substituted aniline.

Polyamines are aliphatic, cycloaliphatic and aromatic polyamines analogous to the above-described monoamines except for the presence within their structure of additional amino nitrogens. The additional amino nitrogens can be primary, secondary or tertiary amino nitrogens. Examples of such polyamines include N-amino-propyl-cyclohexylamines, N,N'-di-n-butyl-paraphenylene diamine, bis-(para-aminophenyl)methane, 1,4-diaminocyclohexane, and the like.

The hydroxy-substituted amines contemplated are those having hydroxy substituents bonded directly to a carbon atom other than a carbonyl carbon atom; that is, they have hydroxy groups capable of functioning as alcohols. Examples of such hydroxy-substituted amines include ethanolamine, di-(3-hydroxypropyl)-amine, 3-hydroxybutyl-amine, 4-hydroxybutyl-amine, diethanolamine, di-(2-hydroxyamine, N-(hydroxypropyl)-propylamine, N-(2-methyl)-cyclohexylamine, 3-hydroxycyclopentyl parahydroxyaniline, N-hydroxyethal piperazine and the like.

In one embodiment, the amines useful in the present invention are alkylene polyamines including hydrogen, or a hydrocarbyl, amino hydrocarbyl, hydroxyhydrocarbyl or heterocyclic-substituted hydrocarbyl group containing up to about 10 carbon atoms, Alk is an alkylene group containing up to about 10 carbon atoms, and is 2 to about 10. Preferably, Alk is ethylene or propylene. Usually, a will have an average value of from 2 to about 7. Examples of such alkylene polyamines include methylene polyamines, ethylene polyamines, butylene polyamines, propylene polyamines, pentylene polyamines, hexylene polyamines, heptylene polyamines, etc.

Alkylene polyamines include ethylene diamine, triethylene tetramine, propylene diamine, trimethylene diamine, hexamethylene diamine, decamethylene diamine, hexamethylene diamine, decamethylene diamine, octamethylene diamine, di(heptamethylene) triamine, tripropylene tetraamine, tetraethylene pentamine, trimethylene diamine, pentethylene hexamine, di(trimethylene)triamine, and the like. Higher homologs as are obtained by condensing two or more of the above-illustrated alkylene amines are useful, as are mixtures of two or more of any of the afore-described polyamines.

Ethylene polyamines, such as those mentioned above, are especially useful for reasons of cost and effectiveness. Such polyamines are described in detail under the heading "Diamines and Higher Amines" in The Encyclopedia of Chemical Technology, Second Edition, Kirk and Othmer, Volume 7, pages 27-39, Interscience Publishers, Division of John Wiley and Sons, 1965, which is hereby incorporated by reference for the disclosure of useful polyamines. Such compounds are prepared most conveniently by the reaction of an alkylene chloride with ammonia or by reaction of an ethylene imine with a ring-opening reagent such as ammonia, etc. These reactions result in the production of the somewhat complex mixtures of alkylene polyamines, including cyclic condensation products such as piperazines.

Other useful types of polyamine mixtures are those resulting from stripping of the above-described polyamine mixtures. In this instance, lower molecular weight polyamines and volatile contaminants are removed from an alkylene polyamine mixture to leave as residue what is often termed "polyamine bottoms". In general, alkylene polyamine bottoms can be characterized as having less than 2, usually less than 1% (by weight) material boiling below about 200 degree C. In the instance of ethylene polyamine bottoms, which are readily available and found to be quite useful, the bottoms contain less than about 2% (by weight) total diethylene triamine (DETA) or triethylene tetramine (TETA). A typical sample such ethylene polyamine bottoms obtained from the Dow Chemical Company of Freeport, Tx. designated "E-100". Gas chromatography analysis of such a sample showed it to contain about 0.93% "Light Ends" (most probably DETA), 0.72% TETA, 21.74% tetraethylene pentamine and 76.61% pentaethylene hexamine and higher (by weight). These alkylene polyamine bottoms include cyclic condensa-

tion products such as piperazine and higher analogs of diethylene triamine, triethylene tetramine and the like.

The dispersants are selected from

5 Mannich bases that are condensation reaction products of a high molecular weight phenol, an alkylene polyamine and an aldehyde such as formaldehyde;

10 succinic-based dispersants that are reaction products of a olefin polymer and succinic acylating agent (acid, anhydride, ester or halide) further reacted with an organic hydroxy compound and/or an amine; and

high molecular weight amides and esters such as reaction products of a hydrocarbyl acylating agent and a polyhydric aliphatic alcohol (such as glycerol, pentaerythritol or sorbitol).

15 Ashless (metal-free) polymeric materials usually contain an oil soluble high molecular weight backbone linked to a polar functional group that associates with particles to be dispersed are typically used as dispersants. Zinc acetate capped, also any treated dispersant, which include borated, 20 cyclic carbonate, end-capped, polyalkylene maleic anhydride and the like; mixtures of some of the above, in treat rates that range from about 0.1% up to 10-20% or more. Commonly used hydrocarbon backbone materials are olefin polymers and copolymers, i.e.—ethylene, propylene, butylene, isobutylene, styrene; there may or may not be further functional groups incorporated into the backbone of the polymer, whose molecular weight ranges from 300 up to 5000. Polar materials such as amines, alcohols, amides or esters are attached to the backbone via a bridge.

25 30 Antioxidants: include sterically hindered alkyl phenols such as 2,6-di-tert-butylphenol, 2,6-di-tert-butyl-p-cresol and 2,6-di-tert-butyl-4-(2-octyl-3-propanoic)phenol; N,N-di(alkylphenyl)amines; and alkylated phenylene-diamines.

35 The antioxidant component may be a hindered phenolic antioxidant such as butylated hydroxytoluene, suitably present in an amount of 0.01 to 5%, preferably 0.4 to 0.8%, by weight of the lubricant composition. Alternatively, or in addition, component b) may comprise an aromatic amine antioxidant such as mono-octylphenylalphanaphthylamine or p,p-diocyldiphenylamine, used singly or in admixture. The amine anti-oxidant component is suitably present in a range of from 0.01 to 5% by weight of the lubricant composition, more preferably 0.5 to 1.5%.

40 45 The amine-type antioxidant includes, for example, monoalkyldiphenylamines such as monoocetyl diphenylamine and monononyldiphenylamine; dialkyldiphenylamines such as 4,4'-dibutyldiphenylamine, 4,4'-dipentyl diphenylamine, 4,4'-dihexyldiphenylamine, 4,4'-diheptyldiphenylamine, 4,4'-diocetyl diphenylamine and 4,4'-dinonyldiphenylamine; 50 polyalkyldiphenylamines such as tetrabutyl diphenylamine, tetrahexyldiphenylamine, tetraoctyldiphenylamine and tetra-nonyldiphenylamine; and naphthylamines such as alpha-naphthylamine, phenyl-alpha-naphthylamine, butylphenyl-alpha-naphthylamine, pentylphenyl-alpha-naphthylamine, 55 hexylphenyl-alpha-naphthylamine, heptylphenyl-alpha-naphthylamine, octylphenyl-alpha-naphthylamine and nonylphenyl-alpha-naphthylamine. Of these, preferred are dialkyldiphenylamines. The sulfur-containing antioxidant and the amine-type antioxidant are added to the base oil in an amount of from 0.01 to 5% by weight, preferably from 0.03 to 3% by weight, relative to the total weight of the composition.

60 65 Oxidation inhibitors, organic compounds containing nitrogen, phosphorus and some alkylphenols are also employed. Two general types of oxidation inhibitors are those that react with the initiators, peroxy radicals, and hydroperoxides to form inactive compounds, and those that decompose these

materials to form less active compounds. Examples are hindered (alkylated) phenols, e.g. 6-di(tert-butyl)-4-methylphenol [2,6-di(tert-butyl)-p-cresol, DBPC], and aromatic amines, e.g. N-phenyl-alpha-naphthalamine. These are used in turbine, circulation, and hydraulic oils that are intended for extended service; with ratios of amine/phenolic to be from 1:10 to 10:1 of the mixtures preferred.

Examples of amine-based antioxidants include dialkyl-diphenylamines such as p,p'-diocylidiphenylamine (manufactured by the Seiko Kagaku Co. under the trade designation "Nonflex OD-3"), p,p'-di-alpha.-methylbenzyl-diphenylamine and N-p-butylphenyl-N-p'-octylphenylamine; monoalkyldiphenylamines such as mono-t-butylidiphenylamine, and monoocetylidiphenylamine; bis(dialkylphenyl) amines such as di(2,4-diethylphenyl)amine and di(2-ethyl-4-nonylphenyl)amine; alkylphenyl-1-naphthylamines such as octylphenyl-1-naphthylamine and N-t-dodecylphenyl-1-naphthylamine; arylnaphthylamines such as 1-naphthylamine, phenyl-1-naphthylamine, phenyl-2-naphthylamine, N-hexylphenyl-2-naphthylamine and N-octylphenyl-2-naphthylamine, phenylenediamines such as N,N'-diisopropyl-p-phenylenediamine and N,N'-diphenyl-p-phenylenediamine.

Examples of phenol-based antioxidants include 2-t-butylphenol, 2-t-butyl-4-methylphenol, 2-t-butyl-5-methylphenol, 2,4-di-t-butylphenol, 2,4-dimethyl-6-t-butylphenol, 2-t-butyl-4-methoxyphenol, 3-t-butyl-4-methoxyphenol, 2,5-di-t-butylhydroquinone (manufactured by the Kawaguchi Kagaku Co. under trade designation "Antage DBH"), 2,6-di-t-butylphenol and 2,6-di-t-butyl-4-alkylphenols such as 2,6-di-t-butyl-4-methylphenol and 2,6-di-t-butyl-4-ethylphenol; and 2,6-di-t-butyl-4-alkoxyphenols such as 2,6-di-t-butyl-4-methoxyphenol and 2,6-di-t-butyl-4-ethoxyphenol, 3,5-di-t-butyl-4-hydroxybenzylmercaptoocty-1 acetate, alkyl-3-(3,5-di-t-butyl-4-hydroxyphenyl)propionates such as n-octyl-3-(3,5-di-t-butyl-4-hydroxyphenyl)propionate (manufactured by Yoshitomi Seiyaku Co. under the trade designation "Yonox SS"), n-dodecyl-3-(3,5-di-t-butyl-4-hydroxyphenyl)propionate and 2'-ethylhexyl-3-(3,5-di-t-butyl-4-hydroxyphenyl)propionate; 2,6-di-t-butyl-alpha.-dimethylamino-p-cresol, 2,2'-methylenebis(4-alkyl-6-t-butylphenol) compounds such as 2,2'-methylenebis(4-methyl-6-t-butylphenol) (manufactured by the Kawaguchi Kagaku Co. under the trade designation "Antage W-400") and 2,2'-methylenebis(4-ethyl-6-t-butylphenol) (manufactured by the Kawaguchi Kagaku Co. under the trade designation "Antage W-500"); bisphenols such as 4,4'-butyldenebis(3-methyl-6-t-butyl-phenol) (manufactured by the Kawaguchi Kagaku Co. under the trade designation "Antage W-300"), 4,4'-methylenebis(2,6-di-t-butylphenol) (manufactured by Laporte Performance Chemicals under the trade designation "Ionox 220AH"), 4,4'-bis(2,6-di-t-butylphenol), 2,2-di-p-hydroxyphenylpropane (Bisphenol A), 2,2-bis(3,5-di-t-butyl-4-hydroxyphenyl)propane, 4,4'-cyclohexylidenebis(2,6-di-t-butylphenol), hexamethylene glycol bis[3,(3,5-di-t-butyl-4-hydroxyphenyl)propionate] (manufactured by the Ciba Specialty Chemicals Co. under the trade designation "Irganox L109"), triethylene glycol bis[3-(3-t-butyl-4-hydroxy-5-methylphenyl)propionate] (manufactured by the Yoshitomi Seiyaku Co. under the trade designation "Tominox 917"), 2,2'-thio[diethyl-3-(3,5-di-t-butyl-4-hydroxyphenyl)propionate] (manufactured by the Ciba Specialty Chemicals Co. under the trade designation "Irganox L115"), 3,9-bis{1,1-dimethyl-2-[3-(3-t-butyl-4-hydroxy-5-methylphenyl)-propionyloxy]ethyl}2,4,8,10-tetraoxaspiro[5,5]undecane (manufactured by the Sumitomo Kagaku Co. under the trade designation "Sumilizer GA80"), 1,1,3-tris(2-methyl-4-hy-

droxy-5-t-butylphenyl)butane (manufactured by the Yoshitomi Seiyaku Co. under the trade designation "Yoshinox 930"), 1,3,5-trimethyl-2,4,6-tris(3,5-di-t-butyl-4-hydroxybenzyl)benzene (manufactured by Ciba Specialty Chemicals under the trade designation "Irganox 330"), bis[3,3'-bis(4'-hydroxy-3'-t-butylphenyl)butyric acid]glycol ester, 2-(3',5'-di-t-butyl-4-hydroxyphenyl)-methyl-4-(2",4"-di-t-butyl-3"-hydroxyphenyl)methyl-6-t-butylphenol and 2,6-bis(2'-hydroxy-3'-t-butyl-5'-methylbenzyl)-4-methylphenol; and phenol/aldehyde condensates such as the condensates of p-t-butylphenol and formaldehyde and the condensates of p-t-butylphenol and acetaldehyde.

Viscosity index improvers and/or the pour point depressant include polymeric alkylmethacrylates and olefinic copolymers such as an ethylenepropylene copolymer or a styrene-butadiene copolymer or polyalkene such as PIB. Viscosity index improvers (VI improvers), high molecular weight polymers that increase the relative viscosity of an oil at high temperatures more than they do at low temperatures. The most common VI improvers are methacrylate polymers and copolymers, acrylate polymers, olefin polymers and copolymers, and styrene-butadiene copolymers.

Other examples of the viscosity index improver include 25 polymethacrylate, polyisobutylene, alpha-olefin polymers, alpha-olefin copolymers (e.g., an ethylene-propylene copolymer), polyalkylstyrene, phenol condensates, naphthalene condensates, a styrenebutadiene copolymer and the like. Of these, polymethacrylate having a number average molecular weight of 10,000 to 300,000, and alpha-olefin polymers or alpha-olefin copolymers having a number average molecular weight of 1,000 to 30,000, particularly ethylene-alpha-olefin copolymers having a number average molecular weight of 1,000 to 10,000 are preferred.

The viscosity index increasing agents which can be used include, for example, polymethacrylates and ethylene/propylene copolymers, other non-dispersion type viscosity index increasing agents such as olefin copolymers like styrene/diene copolymers, and dispersible type viscosity index increasing agents where a nitrogen containing monomer has been copolymerized in such materials. These materials can be added and used individually or in the form of mixtures, conveniently in an amount within the range of from 0.05 to 20 parts by weight per 100 parts by weight of base oil.

45 Pour point depressors (PPD): include polymethacrylates. Commonly used additives such as alkylaromatic polymers and polymethacrylates are useful for this purpose; typically the treat rates range from 0.001% to 1.0%.

Anti-rust additives: include (short-chain) alkenyl succinic acids, partial esters thereof and nitrogen-containing derivatives thereof. Anti-rust agents include, for example, monocarboxylic acids which have from 8 to 30 carbon atoms, alkyl or alkenyl succinates or partial esters thereof, hydroxy-fatty acids which have from 12 to 30 carbon atoms and derivatives 50 thereof, sarcosines which have from 8 to 24 carbon atoms and derivatives thereof, amino acids and derivatives thereof, naphthenic acid and derivatives thereof, lanolin fatty acid, mercapto-fatty acids and paraffin oxides.

Particularly preferred anti-rust agents are indicated below. 55 Examples of Monocarboxylic Acids (C8-C30), Caprylic acid, pelargonic acid, decanoic acid, undecanoic acid, lauric acid, myristic acid, palmitic acid, stearic acid, arachic acid, behenic acid, cerotic acid, montanic acid, melissic acid, oleic acid, docosanic acid, erucic acid, eicosanic acid, beef tallow fatty acid, soy bean fatty acid, coconut oil fatty acid, linolic acid, linoleic acid, tall oil fatty acid, 12-hydroxystearic acid, laurylsarcosinic acid, myritsylsarcosinic acid, palmitylsar-

cosinic acid, stearylsarcosinic acid, oleylsarcosinic acid, alkylated (C8-C20) phenoxyacetic acids, lanolin fatty acids.

Examples of Polybasic Carboxylic Acids: The alkenyl (C10-C100) succinic acids indicated in CAS No. 27859-58-1 and ester derivatives thereof, dimer acid, N-acyl-N-alkyloxy-alkyl aspartic acid esters (U.S. Pat. No. 5,275,749).

Examples of the alkylamines which function as antirust additives or as reaction products with the above carboxylates to give amides and the like are represented by primary amines such as laurylamine, coconut-amine, n-tridecylamine, myristylamine, n-pentadecylamine, palmitylamine, n-heptadecylamine, stearylamine, n-nonadecylamine, n-eicosylamine, n-heneicosylamine, n-docosylamine, n-tricosylamine, n-pentacosylamine, oleylamine, beef tallow-amine, hydrogenated beef tallow-amine and soy bean-amine. Examples of the secondary amines include dilaurylamine, di-coconutamine, di-n-tridecylamine, dimyristylamine, di-n-pentadecylamine, dipalmitylamine, di-n-pentadecylamine, distearylamine, di-n-nonadecylamine, di-n-eicosylamine, di-n-heneicosylamine, di-n-docosylamine, di-n-tricosylamine, di-n-pentacosyl-amine, dioleylamine, di-beef tallow-amine, di-hydrogenated beef tallow-amine and di-soy bean-amine.

Examples of the aforementioned N-alkylpolyalkylenediamines include: ethylenediamines such as laurylethylenediamine, coconut ethylenediamine, n-tridecylethylenediamine-, myristylethylenediamine, n-pentadecylethylenediamine, palmitylethylenediamine, n-heptadecylethylenediamine, stearylethylenediamine, n-nonadecylethylenediamine, n-eicosylethylenediamine, n-heneicosylethylenediamine, n-tricosylethylenediamine, n-pentacosylethylenediamine, oleylethylenediamine, beef tallow-ethylenediamine, hydrogenated beef tallow-ethylenediamine and soy bean-ethylenediamine; propylenediamines such as laurylpropylenediamine, coconut propylenediamine, n-tridecylpropylenediamine, myristylpropylenediamine, n-pentadecylpropylenediamine, palmitylpropylenediamine, n-heptadecylpropylenediamine, stearylpropylenediamine, n-nonadecylpropylenediamine, n-eicosylpropylenediamine, n-heneicosylpropylenediamine, n-docosylpropylenediamine, n-tricosylpropylenediamine, n-pentacosylpropylenediamine, diethylene triamine (DETA) or triethylene tetramine (TETA), oleylpropylenediamine, beef tallow-propylenediamine, hydrogenated beef tallow-propylenediamine and soy bean-propylenediamine; butylenediamines such as laurylbutylenediamine, coconut butylenediamine, n-tridecylbutylenediamine-, myristylbutylenediamine, n-pentadecylbutylenediamine, stearylbutylenediamine, n-eicosylbutylenediamine, n-heneicosylbutylenediamine, n-docosylbutylenediamine, n-tricosylbutylenediamine, n-pentacosylbutylenediamine, oleylbutylenediamine, beef tallow-butylenediamine, hydrogenated beef tallow-butylenediamine and soy bean butylenediamine; and pentylenediamines such as laurylpentylenediamine, coconut pentylenediamine, myristylpentylenediamine, palmitylpentylenediamine, stearylpentylenediamine, oleylpentylenediamine, beef tallow-pentylenediamine, hydrogenated beef tallow-pentylenediamine and soy bean pentylenediamine.

Demulsifying agents: include alkoxylated phenols and phenolformaldehyde resins and synthetic alkylaryl sulfonates such as metallic dinonylnaphthalene sulfonates. A demulsifying agent is a predominant amount of a water-soluble polyoxyalkylene glycol having a pre-selected molecular weight of any value in the range of between about 450 and 5000 or more. An especially preferred family of water soluble polyoxyalkylene glycol useful in the compositions of the present

invention may also be one produced from alkoxylation of n-butanol with a mixture of alkylene oxides to form a random alkoxylated product.

Functional fluids according to the invention possess a pour point of less than about -20 degree C., and exhibit compatibility with a wide range of anti-wear additive and extreme pressure additives. The formulations according to the invention also are devoid of fatigue failure that is normally expected by those of ordinary skill in the art when dealing with polar lubricant base stocks.

Polyoxyalkylene glycols useful in the present invention may be produced by a well-known process for preparing polyalkylene oxide having hydroxyl end-groups by subjecting an alcohol or a glycol ether and one or more alkylene oxide monomers such as ethylene oxide, butylene oxide, or propylene oxide to form block copolymers in addition polymerization while employing a strong base such as potassium hydroxide as a catalyst. In such process, the polymerization is commonly carried out under a catalytic concentration of 0.3 to 1.0% by mole of potassium hydroxide to the monomer(s) and at high temperature, as 100 degrees C. to 160 degrees C. It is well known fact that the potassium hydroxide being a catalyst is for the most part bonded to the chain-end of the produced polyalkylene oxide in a form of alkoxide in the polymer solution so obtained.

An especially preferred family of soluble polyoxyalkylene glycol useful in the compositions of the present invention may also be one produced from alkoxylation of n-butanol with a mixture of alkylene oxides to form a random alkoxylated product.

Foam inhibitors: include polymers of alkyl methacrylate especially useful poly alkyl acrylate polymers where alkyl is generally understood to be methyl, ethyl propyl, isopropyl, butyl, or iso butyl and polymers of dimethylsilicone which form materials called dimethylsiloxane polymers in the viscosity range of 100 cSt to 100,000 cSt. Other additives are defoamers, such as silicone polymers which have been post reacted with various carbon containing moieties, are the most widely used defoamers. Organic polymers are sometimes used as defoamers although much higher concentrations are required.

Metal deactivating compounds/Corrosion inhibitors: include alkyltriazoles and benzotriazoles. Examples of dibasic acids useful as anti-corrosion agents, other than sebacic acids, which may be used in the present invention, are adipic acid, azelaic acid, dodecanedioic acid, 3-methyladipic acid, 3-nitrophthalic acid, 1,10-decanedicarboxylic acid, and fumaric acid. The anti-corrosion combination is a straight or branch-chained, saturated or unsaturated monocarboxylic acid or ester thereof. Preferably the acid is a C sub 4 to C sub 22 straight chain unsaturated monocarboxylic acid. The preferred concentration of this additive is from 0.001% to 0.35% by weight of the total lubricant composition. However, other suitable materials are oleic acid itself; valeric acid and erucic acid. A component of the anti-corrosion combination is a triazole as previously defined. The triazole should be used at a concentration from 0.005% to 0.25% by weight of the total composition. The preferred triazole is tolylotriazole which may be included in the compositions of the invention include triazoles, thiiazoles and certain diamine compounds which are useful as metal deactivators or metal passivators. Examples include triazole, benzotriazole and substituted benzotriazoles such as alkyl substituted derivatives. The alkyl substituent generally contains up to 1.5 carbon atoms, preferable up to 8 carbon atoms. The triazoles may contain other substituents on the aromatic ring such as halogens, nitro, amino, mercapto, etc. Examples of suitable compounds are benzotriazole and

the tolyltriazoles, ethylbenzotriazoles, hexylbenzotriazoles, octylbenzotriazoles and nitrobenzotriazoles. Benzotriazole and tolyltriazole are particularly preferred. A straight or branched chain saturated or unsaturated monocarboxylic acid which is optionally sulphurised in an amount which may be up to 35% by weight; or an ester of such an acid; and a triazole or alkyl derivatives thereof, or short chain alkyl of up to 5 carbon atoms; n is zero or an integer between 1 and 3 inclusive; and is hydrogen, morpholine, alkyl, amido, amino, hydroxy or alkyl or aryl substituted derivatives thereof; or a triazole selected from 1,2,4 triazole, 1,2,3 triazole, 5-anilo-1, 2,3,4-thiatriazole, 3-amino-1,2,4 triazole, 1-H-benzotriazole-1-yl-methylisocyanide, methylene-bis-benzotriazole and naphthotriazole.

Alkyl is straight or branched chain and is for example methyl, ethyl, n-propyl, iso-propyl, n-butyl, sec-butyl, n-pentyl, n-hexyl, n-heptyl, n-octyl, 2-ethylhexyl, n-nonyl, n-decyl, n-dodecyl, n-tetradecyl, n-hexadecyl, n-octadecyl or n-eicosyl.

Alkenyl is straight or branched chain and is for example prop-2-enyl, but-2-enyl, 2-methyl-prop-2-enyl, pent-2-enyl, hexa-2,4-dienyl, dec-10-enyl or eicos-2-enyl.

Cycloalkyl is for example cyclopentyl, cyclohexyl, cyclooctyl, cyclodecyl, adamantyl or cyclododecyl.

Aralkyl is for example benzyl, 2-phenylethyl, benzhydryl or naphthylmethyl.

Aryl is for example phenyl or naphthyl.

The heterocyclic group is for example a morpholine, pyrrolidine, piperidine or a perhydroazepine ring.

Alkylene moieties include for example methylene, ethylene, 1:2- or 1:3-propylene, 1:4-butylene, 1:6-hexylene, 1:8-octylene, 1:10-decylene and 1:12-dodecylene.

Arylene moieties include for example phenylene and naphthylene. 1-(or 4)-(dimethylaminomethyl)triazole, 1-(or 4)-(diethylaminomethyl)triazole, 1-(or 4)-(di-isopropylaminomethyl)triazole, 1-(or 4)-(di-n-butylaminomethyl)triazole, 1-(or 4)-(di-n-hexylaminomethyl)triazole, 1-(or 4)-(di-isooctylaminomethyl)triazole, 1-(or 4)-(di-(2-ethylhexyl)aminomethyl)triazole, 1-(or 4)-(di-n-decylaminomethyl)triazole, 1-(or 4)-(di-n-dodecylaminomethyl)triazole, 1-(or 4)-(di-n-octadecylaminomethyl)triazole, 1-(or 4)-(di-n-eicosylaminomethyl)triazole, 1-(or 4)-[di-(prop-2'-enyl)aminomethyl]triazole, 1-(or 4)-[di-(but-2'-enyl)aminomethyl]triazole, 1-(or 4)-[di-(eicos-2'-enyl)aminomethyl]triazole, 1-(or 4)-(di-cyclohexylaminomethyl)triazole, 1-(or 4)-(di-benzylaminomethyl)triazole, 1-(or 4)-(di-phenylaminomethyl)triazole, 1-(or 4)-(4'-morpholinomethyl)triazole, 1-(or 4)-(1'-pyrrolidinomethyl)triazole, 1-(or 4)-(1'-perhydroazepinomethyl)triazole, 1-(or 4)-(2',2"-dihydroxyethyl)aminomethyl]triazole, 1-(or 4)-(dibutoxypropyl-aminomethyl)triazole, 1-(or 4)-(dibutylthiopropyl-aminomethyl)triazole, 1-(or 4)-(dibutylaminopropyl-aminomethyl)triazole, 1-(or 4)-(1-methanomine)-N,N-bis(2-ethylhexyl)-methyl benzotriazole, N,N-bis-(1- or 4-triazolylmethyl)laurylamine, N,N-bis-(1- or 4-triazolylmethyl)oleylamine, N,N-bis-(1- or 4-triazolylmethyl)ethanolamine and N,N,N',N'-tetra(1- or 4-triazolylmethyl)ethylene diamine.

The metal deactivating agents which can be used in the lubricating oil a composition of the present invention include benzotriazole and the 4-alkylbenzotriazoles such as 4-methylbenzotriazole and 4-ethylbenzotriazole; 5-alkylbenzotriazoles such as 5-methylbenzotriazole, 5-ethylbenzotriazole; 1-alkylbenzotriazoles such as 1-dioctylauainomethyl-2,3-benzotriazole; benzotriazole derivatives such as the 1-alkyltolutriazoles, for example, 1-dioctylaminomethyl-2,3-tolu-

triazole; benzimidazole and benzimidazole derivatives or concentrates and/or mixtures thereof.

Anti-wear agents/Extreme pressure agent/Friction Reducer: aryl phosphates and phosphites, and metal or ash-free carbamates.

5 A phosphate ester or salt may be a monohydrocarbyl, dihydrocarbyl or a trihydrocarbyl phosphate, wherein each hydrocarbyl group is saturated. In one embodiment, each hydrocarbyl group independently contains from about 8 to about 30, or from about 12 up to about 28, or from about 14 up to about 24, or from about 14 up to about 18 carbons atoms. In one embodiment, the hydrocarbyl groups are alkyl groups. Examples of hydrocarbyl groups include tridecyl, tetradecyl, pentadecyl, hexadecyl, heptadecyl, octadecyl groups and mixtures thereof.

10 A phosphate ester or salt is a phosphorus acid ester prepared by reacting one or more phosphorus acid or anhydride with a saturated alcohol. The phosphorus acid or anhydride is generally an inorganic phosphorus reagent, such as phosphorus pentoxide, phosphorus trioxide, phosphorus tetroxide, phosphorous acid, phosphoric acid, phosphorus halide, lower phosphorus esters, or a phosphorus sulfide, including phosphorus pentasulfide, and the like. Lower phosphorus acid esters generally contain from 1 to about 7 carbon atoms in each ester group. Alcohols used to prepare the phosphorus acid esters or salts.

15 Examples of commercially available alcohols and alcohol mixtures include Alfol 1218 (a mixture of synthetic, primary, straight-chain alcohols containing 12 to 18 carbon atoms); Alfol20+ alcohols (mixtures of C18-C28 primary alcohols having mostly C20 alcohols as determined by GLC (gas-liquid-chromatography)); and Alfol22+ alcohols (C18-C28 primary alcohols containing primarily C22 alcohols). Alfol 20 alcohols are available from Continental Oil Company. Another example of a commercially available alcohol mixture is Adol 60 (about 75% by weight of a straight chain C22 primary alcohol, about 15% of a C20 primary alcohol and about 8% of C18 and C24 alcohols). The Adol alcohols are marketed by Ashland Chemical.

20 A variety of mixtures of monohydric fatty alcohols derived from naturally occurring triglycerides and ranging in chain length from C8 to C18 are available from Procter & Gamble Company. These mixtures contain various amounts of fatty alcohols containing 12, 14, 16, or 18 carbon atoms. For example, CO-1214 is a fatty alcohol mixture containing 0.5% of C10 alcohol, 66.0% of C12 alcohol, 26.0% of C14 alcohol and 6.5% of C16 alcohol.

25 Another group of commercially available mixtures include the "Neodol" products available from Shell Chemical Co. For example, Neodol 23 is a mixture of C12 and C13 alcohols; Neodol 25 is a mixture of C12 to C15 alcohols; and Neodol 45 is a mixture of C14 to C15 linear alcohols. The phosphate contains from about 14 to about 18 carbon atoms in each hydrocarbyl group. The hydrocarbyl groups of the phosphate are generally derived from a mixture of fatty alcohols having from about 14 up to about 18 carbon atoms. The hydrocarbyl phosphate may also be derived from a fatty vicinal diol. Fatty vicinal diols include those available from Ashland Oil under 30 the general trade designation Adol 114 and Adol 158. The former is derived from a straight chain alpha olefin fraction of C11-C14, and the latter is derived from a C15-C18 fraction.

35 The phosphate salts may be prepared by reacting an acidic phosphate ester with an amine compound or a metallic base to form an amine or a metal salt. The amines may be monoamines or polyamines. Useful amines include those amines disclosed in U.S. Pat. No. 4,234,435.

The monoamines generally contain a hydrocarbyl group which contains from 1 to about 30 carbon atoms, or from 1 to about 12, or from 1 to about 6. Examples of primary monoamines useful in the present invention include methylamine, ethylamine, propylamine, butylamine, cyclopentylamine, cyclohexylamine, octylamine, dodecylamine, allylamine, cocoamine, stearylamine, and laurylamine. Examples of secondary monoamines include dimethylamine, diethylamine, dipropylamine, dibutylamine, dicyclopentylamine, dicyclohexylamine, methylbutylamine, ethylhexylamine, etc.

An amine is a fatty (C<sub>sub.8-30</sub>) amine which includes n-octylamine, n-decylamine, n-dodecylamine, n-tetradecylamine, n-hexadecylamine, n-octadecylamine, oleyamine, etc. Also useful fatty amines include commercially available fatty amines such as "Armeen" amines (products available from Akzo Chemicals, Chicago, Ill.), such Armeen C, Armeen O, Armeen O L, Armeen T, Armeen H T, Armeen S and Armeen S D, wherein the letter designation relates to the fatty group, such as coco, oleyl, tallow, or stearyl groups.

Other useful amines include primary ether amines, such as those represented by the formula, R<sup>"</sup>(OR')<sub>x</sub>NH<sub>2</sub>, wherein R' is a divalent alkylene group having about 2 to about 6 carbon atoms; x is a number from one to about 150, or from about one to about five, or one; and R" is a hydrocarbyl group of about 5 to about 150 carbon atoms. An example of an ether amine is available under the name SURFAM® amines produced and marketed by Mars Chemical Company, Atlanta, Ga. Preferred etheramines are exemplified by those identified as SURFAM P14B (decyloxypropylamine), SURFAM P16A (linear C 16), SURFAM P17B (tridecyloxypropylamine). The carbon chain lengths (i.e., C 14, etc.) of the SURFAMS described above and used hereinafter are approximate and include the oxygen ether linkage.

An amine is a tertiary-aliphatic primary amine. Generally, the aliphatic group, preferable an alkyl group, contains from about 4 to about 30, or from about 6 to about 24, or from about 8 to about 22 carbon atoms. Usually the tertiary alkyl primary amines are monoamines the alkyl group is a hydrocarbyl group containing from one to about 27 carbon atoms and R<sub>6</sub> is a hydrocarbyl group containing from 1 to about 12 carbon atoms. Such amines are illustrated by tert-butylamine, tert-hexylamine, 1-methyl-1-amino-cyclohexane, tert-octylamine, tert-decylamine, tert-dodecylamine, tert-tetradecylamine, tert-hexadecylamine, tert-octadecylamine, tert-tetracosanylamine, and tert-octacosanylamine. Mixtures of tertiary aliphatic amines may also be used in preparing the phosphate salt. Illustrative of amine mixtures of this type are "Primene 81R" which is a mixture of C11-C14 tertiary alkyl primary amines and "Primene JMT" which is a similar mixture of C18-C<sub>22</sub> tertiary alkyl primary amines (both are available from Rohm and Haas Company). The tertiary aliphatic primary amines and methods for their preparation are known to those of ordinary skill in the art. The tertiary aliphatic primary amine useful for the purposes of this invention and methods for their preparation are described in U.S. Pat. An amine is a heterocyclic polyamine. The heterocyclic polyamines include aziridines, azetidines, azolidines, tetra- and dihydropyridines, pyrroles, indoles, piperidines, imidazoles, di- and tetra-hydroimidazoles, piperazines, isoindoles, purines, morpholines, thiomorpholines, N-aminoalkylmorpholines, N-aminoalkylthiomorpholines, N-aminoalkyl-piperazines, N,N'-diaminoalkylpiperazines, azepines, azocines, azonines, azecines and tetra-, di- and perhydro derivatives of each of the above and mixtures of two or more of these heterocyclic amines. Preferred heterocyclic amines are the saturated 5- and 6-membered heterocyclic amines containing only nitrogen, oxygen and/or sulfur in the hetero ring, espe-

cially the piperidines, piperazines, thiomorpholines, morpholines, pyrrolidines, and the like. Piperidine, aminoalkyl substituted piperidines, piperazine, aminoalkyl substituted piperazines, morpholine, aminoalkyl substituted morpholines, pyrrolidine, and aminoalkyl-substituted pyrrolidines, are especially preferred. Usually the aminoalkyl substituents are substituted on a nitrogen atom forming part of the hetero ring. Specific examples of such heterocyclic amines include N-aminoalkylmorpholine, N-aminoethylpiperazine, and N,N'-diaminoethylpiperazine. Hydroxy heterocyclic polyamines are also useful. Examples include N-(2-hydroxyethyl)cyclohexylamine, 3-hydroxycyclopentylamine, parahydroxyaniline, N-hydroxyethylpiperazine, and the like.

Lubricating compositions also may include a fatty imidazoline or a reaction product of a fatty carboxylic acid and at least one polyamine. The fatty imidazoline has fatty substituents containing from 8 to about 30, or from about 12 to about 24 carbon atoms. The substituent may be saturated or unsaturated, heptadecenyl derived oleyl groups, preferably saturated. In one aspect, the fatty imidazoline may be prepared by reacting a fatty carboxylic acid with a polyalkylenepolyamine, such as those discussed above. The fatty carboxylic acids are generally mixtures of straight and branched chain fatty carboxylic acids containing about 8 to about 30 carbon atoms, or from about 12 to about 24, or from about 16 to about 18. Carboxylic acids include the polycarboxylic acids or carboxylic acids or anhydrides having from 2 to about 4 carbonyl groups, preferably 2. The polycarboxylic acids include succinic acids and anhydrides and Diels-Alder reaction products of unsaturated monocarboxylic acids with unsaturated carboxylic acids (such as acrylic, methacrylic, maleic, fumaric, crotonic and itaconic acids). Preferably, the fatty carboxylic acids are fatty monocarboxylic acids, having from about 8 to about 30, preferably about 12 to about 24 carbon atoms, such as octanoic, oleic, stearic, linoleic, dodecanoic, and tall oil acids, preferably stearic acid. The fatty carboxylic acid is reacted with at least one polyamine. The polyamines may be aliphatic, cycloaliphatic, heterocyclic or aromatic. Examples of the polyamines include alkylene polyamines and heterocyclic polyamines.

Hydroxyalkyl groups are to be understood as meaning, for example, monoethanolamine, diethanolamine or triethanolamine, and the term amine also includes diamine. The amine used for the neutralization depends on the phosphoric esters used. The EP additive according to the invention has the following advantages: It very high effectiveness when used in low concentrations and it is free of chlorine. For the neutralization of the phosphoric esters, the latter are taken and the corresponding amine slowly added with stirring. The resulting heat of neutralization is removed by cooling. The EP additive according to the invention can be incorporated into the respective base liquid with the aid of fatty substances (e.g. tall oil fatty acid, oleic acid, etc.) as solubilizers. The base liquids used are napthenic or paraffinic base oils, synthetic oils (e.g. polyglycols, mixed polyglycols), polyolefins, carboxylic esters, etc.

The composition comprises at least one phosphorus containing extreme pressure additive. Examples of such additives are amine phosphate extreme pressure additives such as that known under the trade name IRGALUBE 349. Such amine phosphates are suitably present in an amount of from 0.01 to 2%, preferably 0.2 to 0.6% by weight of the lubricant composition.

At least one straight and/or branched chain saturated or unsaturated monocarboxylic acid which is optionally sulphurised in an amount which may be up to 35% by weight; and/or an ester of such an acid. At least one triazole or alkyl deriva-

tives thereof, or short chain alkyl of up to 5 carbon atoms and is hydrogen, morphilino, alkyl, amido, amino, hydroxy or alkyl or aryl substituted derivatives thereof; or a triazole selected from 1,2,4 triazole, 1,2,3 triazole, 3-amino-1,2,4 triazole, 1-H-benzotriazole-1-yl-methylisocyanide, methylene-bis-benzotriazole and naphthotriazole; and The neutral organic phosphate which forms a component of the formulation may be present in an amount of 0.01 to 4%, preferably 1.5 to 2.5% by weight of the composition. The above amine phosphates and any of the aforementioned benzo- or tolyl-triazoles can be mixed together to form a single component capable of delivering antiwear performance. The neutral organic phosphate is also a conventional ingredient of lubricating compositions and any such neutral organic phosphate falling within the formula as previously defined may be employed.

Phosphates for use in the present invention include phosphates, acid phosphates, phosphites and acid phosphites. The phosphates include triaryl phosphates, trialkyl phosphates, trialkylaryl phosphates, triarylkyl phosphates and trialkenyl phosphates. As specific examples of these, referred to are triphenyl phosphate, tricresyl phosphate, benzylidiphenyl phosphate, ethyldiphenyl phosphate, tributyl phosphate, ethylidibutyl phosphate, cresyldiphenyl phosphate, dicesylphenyl phosphate, ethylphenyldiphenyl phosphate, diethylphenylphenyl phosphate, propylphenyldiphenyl phosphate, dipropylphenylphenyl phosphate, triethylphenyl phosphate, tripropylphenyl phosphate, butylphenyldiphenyl phosphate, dibutylphenylphenyl phosphate, tributylphenyl phosphate, trihexyl phosphate, tri(2-ethylhexyl)phosphate, tridecyl phosphate, trilauryl phosphate, trimyristyl phosphate, tripalmityl phosphate, tristearyl phosphate, and trioleyl phosphate. The acid phosphates include, for example, 2-ethylhexyl acid phosphate, ethyl acid phosphate, butyl acid phosphate, oleyl acid phosphate, tetracosyl acid phosphate, isodecyl acid phosphate, lauryl acid phosphate, tridecyl acid phosphate, stearyl acid phosphate, and isostearyl acid phosphate.

The phosphites include, for example, triethyl phosphite, tributyl phosphite, triphenyl phosphite, tricresyl phosphite, tri(nonylphenyl)phosphite, tri(2-ethylhexyl)phosphite, tridecyl phosphite, trilauryl phosphite, triisoctyl phosphite, diphenylisodecyl phosphite, tristearyl phosphite, and trioleyl phosphite.

The acid phosphites include, for example, dibutyl hydrogenphosphite, dilauryl hydrogenphosphite, dioleyl hydrogenphosphite, distearyl hydrogenphosphite, and diphenyl hydrogenphosphite.

Amines that form amine salts with such phosphates include, for example, mono-substituted amines, di-substituted amines and tri-substituted amines.

Examples of the mono-substituted amines include butylamine, pentylamine, hexylamine, cyclohexylamine, octylamine, laurylamine, stearylamine, oleylamine and benzylamine; and those of the di-substituted amines include dibutylamine, dipentylamine, dihexylamine, dicyclohexylamine, dioctylamine, dilaurylamine, distearylamine, dioleylamine, dibenzylamine, stearyl monoethanolamine, decyl monoethanolamine, hexyl monopropanolamine, benzyl monoethanolamine, phenyl monoethanolamine, and tolyl monopropanolamine. Examples of tri-substituted amines include tributylamine, tripentylamine, trihexylamine, tricyclohexylamine, trioctylamine, trilaurylamine, tristearylamine, trioleylamine, tribenzylamine, dioleyl monoethanolamine, dilauryl monopropanolamine, dioctyl monoethanolamine, dihexyl monopropanolamine, dibutyl monopropanolamine, oleyl diethanolamine, stearyl dipro-

panolamine, lauryl diethanolamine, octyl dipropanolamine, butyl diethanolamine, benzyl diethanolamine, phenyl diethanolamine, tolyl dipropanolamine, xylyl diethanolamine, triethanolamine, and tripropanolamine.

5 Phosphates are their amine salts are added to the base oil in an amount of from 0.03 to 5% by weight, preferably from 0.1 to 4% by weight, relative to the total weight of the composition.

Carboxylic acids to be reacted with amines include, for 10 example, aliphatic carboxylic acids, dicarboxylic acids (dibasic acids), and aromatic carboxylic acids. The aliphatic carboxylic acids have from 8 to 30 carbon atoms, and may be saturated or unsaturated, and linear or branched. Specific examples of the aliphatic carboxylic acids include pelargonic acid, lauric acid, tridecanoic acid, myristic acid, palmitic acid, stearic acid, isostearic acid, eicosanoic acid, behenic acid, triacontanoic acid, caproic acid, undecylenic acid, oleic acid, linolenic acid, erucic acid, and linoleic acid. Specific examples of the dicarboxylic acids include octadecylsuccinic acid, octadecylsuccinic acid, adipic acid, azelaic acid, and sebamic acid. One example of the aromatic carboxylic acids is salicylic acid. The amines to be reacted with carboxylic acids include for example, polyalkylene-polyamines such as diethylenetriamine, triethylenetetraamine, 15 tetraethylenepentamine, pentaethylenehexamine, hexaethyleneheptamine, heptatethyleneoctamine, dipropylenetriamine, 20 tetrapropylenepentamine, and hexabutyleneheptamine; and alkanolamines such as monoethanolamine and diethanolamine. Of these, preferred are a combination of isostearic acid and tetraethylenepentamine, and a combination of oleic acid 25 and diethanolamine. The reaction products of carboxylic acids and amines are added to the base oil in an amount of from 0.01 to 5% by weight, preferably from 0.03 to 3% by weight, relative to the total weight of the composition.

30 Important components are phosphites. As used herein, the term "hydrocarbyl substituent" or "hydrocarbyl group" is used in its ordinary sense, which is well-known to those skilled in the art. Specifically, it refers to a group having a carbon atom directly attached to the remainder of the molecule and having predominantly hydrocarbon character. Examples of hydrocarbyl groups include:

35 Hydrocarbon substituents, that is, aliphatic (e.g., alkyl or alkenyl), alicyclic (e.g., cycloalkyl, cycloalkenyl) substituents, and aromatic-, aliphatic-, and alicyclic-substituted aromatic substituents, as well as cyclic substituents wherein the ring is completed through another portion of the molecule (e.g., two substituents together form an alicyclic radical); The substituted hydrocarbon substituents, that is, substituents containing non-hydrocarbon groups which, in the context of this invention, do not alter the predominantly hydrocarbon substituent, hydroxy, alkoxy, nitro);

40 Hetero-atom containing substituents, that is, substituents which, while having a predominantly hydrocarbon character, in the context of this invention, contain other than carbon in a ring or chain otherwise composed of carbon atoms. Heteroatoms include sulfur, oxygen, nitrogen, and encompass substituents as pyridyl, furyl, thienyl and imidazolyl. In general, no more than two, preferably no more than one, non-hydrocarbon substituent will be present for every ten carbon atoms 45 in the hydrocarbyl group; typically, there will be no non-hydrocarbon substituents in the hydrocarbyl group.

45 The term "hydrocarbyl group," in the context of the present invention, is also intended to encompass cyclic hydrocarbyl or hydrocarbylene groups, where two or more of the alkyl groups in the above structures together form a cyclic structure. The hydrocarbyl or hydrocarbylene groups of the present invention generally are alkyl or cycloalkyl groups

which contain at least 3 carbon atoms. Preferably or optimally containing sulfur, nitrogen, or oxygen, they will contain 4 to 24, and alternatively 5 to 18 carbon atoms. In another embodiment they contain about 6, or exactly 6 carbon atoms. The hydrocarbyl groups can be tertiary or preferably primary or secondary groups; in one embodiment the component is a di(hydrocarbyl)hydrogen phosphite and each of the hydrocarbyl groups is a primary alkyl group; in another embodiment the component is a di(hydrocarbyl)hydrogen phosphite and each of the hydrocarbyl groups is a secondary alkyl group. In yet another embodiment the component is a hydrocarbylenehydrogen phosphite.

Examples of straight chain hydrocarbyl groups include methyl, ethyl, n-propyl, n-butyl, n-hexyl, n-octyl, n-decyl, n-dodecyl, n-tetradecyl, stearyl, n-hexadecyl, n-octadecyl, oleyl, and cetyl. Examples of branched-chain hydrocarbon groups include isopropyl, isobutyl, secondary butyl, tertiary butyl, neopentyl, 2-ethylhexyl, and 2,6-dimethylheptyl. Examples of cyclic groups include cyclobutyl, cyclopentyl, methylcyclopentyl, cyclohexyl, methylcyclohexyl, cycloheptyl, and cyclooctyl. A few examples of aromatic hydrocarbyl groups and mixed aromatic-aliphatic hydrocarbyl groups include phenyl, methylphenyl, tolyl, and naphthyl.

The R groups can also comprise a mixture of hydrocarbyl groups derived from commercial alcohols. Examples of some monohydric alcohols and alcohol mixtures include the commercially available "Alfol<sup>TM</sup>" alcohols marketed by Continental Oil Corporation. Alfol<sup>TM</sup> 810, for instance, is a mixture containing alcohols consisting essentially of straight chain, primary alcohols having from 8 to 12 carbon atoms. Alfol<sup>TM</sup> 12 is a mixture of mostly C12 fatty alcohols; Alfol<sup>TM</sup> 22+ comprises C18-28 primary alcohols having mostly C22 alcohols, and so on. Various mixtures of monohydric fatty alcohols derived from naturally occurring triglycerides and ranging in chain length from C8 to C18 are available from Procter & Gamble Company. "Neodol<sup>TM</sup>" alcohols are available from Shell Chemical Co., where, for instance, Neodol<sup>TM</sup> 25 is a mixture of C12 to C15 alcohols.

Specific examples of some of the phosphites within the scope of the invention include phosphorous acid, mono-, di-, or tri-propyl phosphite; mono-, di-, or tri-butyl phosphite, di-, or tri-amyl phosphite; mono-, di-, or tri-hexyl phosphite; mono-, di-, or tri-phenyl; mono-, di-, or tri-tolyl phosphite; mono-, di-, or tri-cresyl phosphite; dibutyl phenyl phosphite or mono-, di-, or tri-phosphite, amyl dicesyl phosphite.

The phosphorus compounds of the present invention are prepared by well known reactions. One route the reaction of an alcohol or a phenol with phosphorus trichloride or by a transesterification reaction. Alcohols and phenols can be reacted with phosphorus pentoxide to provide a mixture of an alkyl or aryl phosphoric acid and a dialkyl or diaryl phosphoric acid. Alkyl phosphates can also be prepared by the oxidation of the corresponding phosphites. In any case, the reaction can be conducted with moderate heating. Moreover, various phosphorus esters can be prepared by reaction using other phosphorus esters as starting materials. Thus, medium chain (C9 to C22) phosphorus esters have been prepared by reaction of dimethylphosphite with a mixture of medium-chain alcohols by means of a thermal transesterification or an acid- or base-catalyzed transesterification; see for example U.S. Pat. No. 4,652,416. Most such materials are also commercially available; for instance, triphenyl phosphite is available from Albright and Wilson as Duraphos TPP<sup>TM</sup>; di-n-butyl hydrogen phosphite from Albright and Wilson as Duraphos DBHP<sup>TM</sup>; and triphenylthiophosphate from Ciba Specialty Chemicals as Irgalube TPPT<sup>TM</sup>.

The other major component of the present composition is a hydrocarbon having ethylenic unsaturation. This would normally be described as an olefin or a diene, triene, polyene, and so on, depending on the number of ethylenic unsaturations present. Preferably the olefin is mono unsaturated, that is, containing only a single ethylenic double bond per molecule. The olefin can be a cyclic or a linear olefin. If a linear olefin, it can be an internal olefin or an alpha-olefin. The olefin can also contain aromatic unsaturation, i.e., one or more aromatic rings, provided that it also contains ethylenic (non-aromatic) unsaturation.

The olefin normally will contain 6 to 30 carbon atoms. Olefins having significantly fewer than 6 carbon atoms tend to be volatile liquids or gases which are not normally suitable for formulation into a composition suitable as an antiwear lubricant. Preferably the olefin will contain 6 to 18 or 6 to 12 carbon atoms, and alternatively 6 or 8 carbon atoms.

Among suitable olefins are alkyl-substituted cyclopentenes, hexenes, cyclohexene, alkyl-substituted cyclohexenes, heptenes, cycloheptenes, alkyl-substituted cycloheptenes, octenes including diisobutylene, cyclooctenes, alkyl-substituted cyclooctenes, nonenes, decenes, undecenes, dodecenes including propylene tetramer, tridecenes, tetradecenes, pentadecenes, hexadecenes, heptadecenes, octadecenes, cyclooctadiene, norbornene, dicyclopentadiene, squalene, diphenylacetylene, and styrene. Highly preferred olefins are cyclohexene and 1-octene.

The mixtures of alcohols may be mixtures of different primary alcohols, mixtures of different secondary alcohols or mixtures of primary and secondary alcohols. Examples of useful mixtures include: n-butanol and n-octanol; n-pentanol and 2-ethyl-1-hexanol; isobutanol and n-hexanol; isobutanol and isoamyl alcohol; isopropanol and 2-methyl-4-pentanol; isopropanol and sec-butyl alcohol; isopropanol and isoctyl alcohol; and the like.

Organic triesters of phosphorus acids are also employed in lubricants. Typical esters include triarylphosphates, trialkyl phosphates, neutral alkylaryl phosphates, alkoxyalkyl phosphates, triaryl phosphite, trialkylphosphite, neutral alkyl aryl phosphites, neutral phosphonate esters and neutral phosphine oxide esters. In one embodiment, the long chain dialkyl phosphonate esters are used. More preferentially, the dimethyl-, diethyl-, and dipropyl-oleyl phosphonates can be used. Neutral acids of phosphorus acids are the triesters rather than an acid (HO—P) or a salt of an acid.

Any C4 to C8 alkyl or higher phosphate ester may be employed in the invention. For example, tributyl phosphate (TBP) and tri isoctyl phosphate (TOF) can be used. The specific triphosphate ester or combination of esters can easily be selected by one skilled in the art to adjust the density, viscosity etc. of the formulated fluid. Mixed esters, such as dibutyl octyl phosphate or the like may be employed rather than a mixture of two or more trialkyl phosphates.

A trialkyl phosphate is often useful to adjust the specific gravity of the formulation, but it is desirable that the specific trialkyl phosphate be a liquid at low temperatures. Consequently, a mixed ester containing at least one partially alkylated with a C3 to C4 alkyl group is very desirable, for example 4-isopropylphenyl diphenyl phosphate or 3-butyphenyl diphenyl phosphate. Even more desirable is a triaryl phosphate produced by partially alkylating phenol with butylene or propylene to form a mixed phenol which is then reacted with phosphorus oxychloride as taught in U.S. Pat. No. 3,576,923.

Any mixed triaryl phosphate (TAP) esters may be used as cresyl diphenyl phosphate, tricresyl phosphate, mixed xylyl cresyl phosphates, lower alkylphenyl/phenyl phosphates,

such as mixed isopropylphenyl/phenyl phosphates, t-butylphenyl phenyl phosphates. These esters are used extensively as plasticizers, functional fluids, gasoline additives, flame-retardant additives and the like.

The phosphoric acid ester, thiophosphoric acid ester, and amine salt thereof functions to enhance the lubricating performances, and can be selected from known compounds conventionally employed as extreme pressure agents. Generally employed are phosphoric acid esters, or an amine salt thereof which has an alkyl group, an alkenyl group, an alkylaryl group, or an aralkyl group, any of which contains approximately 3 to 30 carbon atoms.

Examples of the phosphoric acid esters include aliphatic phosphoric acid esters such as triisopropyl phosphate, tributyl phosphate, ethyl dibutyl phosphate, trihexyl phosphate, tri-2-ethylhexyl phosphate, trilauryl phosphate, tristearyl phosphate, and trioleyl phosphate; and aromatic phosphoric acid esters such as benzyl phenyl phosphate, allyl diphenyl phosphate, triphenyl phosphate, tricresyl phosphate, ethyl diphenyl phosphate, cresyl diphenyl phosphate, dicresyl phenyl phosphate, ethylphenyl diphenyl phosphate, diethylphenyl phenyl phosphate, propylphenyl diphenyl phosphate, dipropylphenyl phenyl phosphate, triethylphenyl phosphate, tripropylphenyl phosphate, butylphenyl diphenyl phosphate, dibutylphenyl phenyl phosphate, and tributylphenyl phosphate. Preferably, the phosphoric acid ester is a trialkylphenyl phosphate.

Also employable are amine salts of the above-mentioned phosphates. Amine salts of acidic alkyl or aryl esters of the phosphoric acid and thiophosphoric acid are also employable. Preferably, the amine salt is an amine salt of trialkylphenyl phosphate or an amine salt of alkyl phosphate.

One or any combination of the compounds selected from the group consisting of a phosphoric acid ester, and an amine salt thereof may be used.

The phosphorus acid ester and/or its amine salt function to enhance the lubricating performances, and can be selected from known compounds conventionally employed as extreme pressure agents. Generally employed are a phosphorus acid ester or an amine salt thereof which has an alkyl group, an alkenyl group, an alkylaryl group, or an aralkyl group, any of which contains approximately 3 to 30 carbon atoms.

Examples of the phosphorus acid esters include aliphatic phosphorus acid esters such as triisopropyl phosphite, tributyl phosphite, ethyl dibutyl phosphite, trihexyl phosphite, tri-2-ethylhexylphosphite, trilauryl phosphite, tristearyl phosphite, and trioleyl phosphite; and aromatic phosphorus acid esters such as benzyl phenyl phosphite, allyl diphenylphosphite, triphenyl phosphite, tricresyl phosphite, ethyl diphenyl phosphite, tributyl phosphite, ethyl dibutyl phosphite, cresyl diphenyl phosphite, dicresyl phenyl phosphite, ethylphenyl diphenyl phosphite, diethylphenyl phenyl phosphite, propylphenyl diphenyl phosphite, dipropylphenyl phenyl phosphite, triethylphenyl phosphite, tripropylphenyl phosphite, butylphenyl diphenyl phosphite, dibutylphenyl phenyl phosphite, and tributylphenyl phosphite. Also favorably employed are dilauryl phosphite, dioleyl phosphite, dialkyl phosphites, and diphenyl phosphite. Preferably, the phosphorus acid ester is a dialkyl phosphite or a trialkyl phosphite.

The phosphate salt may be derived from a polyamine. The polyamines include alkoxyLATED diamines, fatty polyamine diamines, alkylenepolyamines, hydroxy containing polyamines, condensed polyamines arylpolyamines, and heterocyclic polyamines. Commercially available examples of alkoxyLATED diamines include those amine where y in the above formula is one. Examples of these amines include

Ethoduomeen T/13 and T/20 which are ethylene oxide condensation products of N-tallowtrimethylenediamine containing 3 and 10 moles of ethylene oxide per mole of diamine, respectively.

In another embodiment, the polyamine is a fatty diamine. The fatty diamines include mono- or dialkyl, symmetrical or asymmetrical ethylene diamines, propane diamines (1,2, or 1,3), and polyamine analogs of the above. Suitable commercial fatty polyamines are Duomeen C. (N-coco-1,3-diaminopropane), Duomeen S (N-soya-1,3-diaminopropane), Duomeen T (N-tallow-1,3-diaminopropane), and Duomeen O (N-oleyl-1,3-diaminopropane). "Duomeens" are commercially available from Armak Chemical Co., Chicago, Ill.

Such alkylenepolyamines include methylenepolyamines, ethylenepolyamines, butylenepolyamines, propylenepolyamines, pentylenepolyamines, etc. The higher homologs and related heterocyclic amines such as piperazines and N-amino alkyl-substituted piperazines are also included. Specific examples of such polyamines are ethylenediamine, triethylenetetramine, tris-(2-aminoethyl)amine, propylenediamine, trimethylenediamine, tripropylenetetramine, tetraethylenepentamine, hexaethyleneheptamine, pentaethylenehexamine, etc. Higher homologs obtained by condensing two or more of the above-noted alkyleneamines are similarly useful as are mixtures of two or more of the aforescribed polyamines.

In one embodiment the polyamine is an ethylenepolyamine. Such polyamines are described in detail under the heading Ethylene Amines in Kirk Othmer's "Encyclopedia of Chemical Technology", 2d Edition, Vol. 7, pages 22-37, Interscience Publishers, New York (1965). Ethylenepolyamines are often a complex mixture of polyalkylenepolyamines including cyclic condensation products.

Other useful types of polyamine mixtures are those resulting from stripping of the above-described polyamine mixtures to leave, as residue, what is often termed "polyamine bottoms". In general, alkylenepolyamine bottoms can be characterized as having less than 2%, usually less than 1% (by weight) material boiling below about 200 C. A typical sample of such ethylene polyamine bottoms obtained from the Dow Chemical Company of Freeport, Tex. designated "E-100". These alkylenepolyamine bottoms include cyclic condensation products such as piperazine and higher analogs of diethylenetriamine, triethylenetetramine and the like. These alkylenepolyamine bottoms can be reacted solely with the acylating agent or they can be used with other amines, polyamines, or mixtures thereof. Another useful polyamine is a condensation reaction between at least one hydroxy compound with at least one polyamine reactant containing at least one primary or secondary amino group. The hydroxy compounds are preferably polyhydric alcohols and amines. The polyhydric alcohols are described below. (See carboxylic ester dispersants.) In one embodiment, the hydroxy compounds are polyhydric amines. Polyhydric amines include any of the above-described monoamines reacted with an alkylene oxide (e.g., ethylene oxide, propylene oxide, butylene oxide, etc.) having from two to about 20 carbon atoms, or from two to about four. Examples of polyhydric amines include tri-(hydroxypropyl)amine, tris-(hydroxymethyl) amino methane, 2-amino-2-methyl-1,3-propanediol, N,N,N',N'-tetrakis(2-hydroxypropyl)ethylenediamine, and N,N,N',N'-tetrakis(2-hydroxyethyl)ethylenediamine, preferably tris(hydroxymethyl)aminomethane (THAM).

Polyamines which react with the polyhydric alcohol or amine to form the condensation products or condensed amines, are described above. Preferred polyamines include triethylenetetramine (TETA), tetraethylenepentamine

41

(TEPA), pentaethylenehexamine (PEHA), and mixtures of polyamines such as the above-described "amine bottoms".

These extreme pressure additives can be used individually or in the form of mixtures, conveniently in an amount within the range from 0.1 to 2 parts by weight, per 100 parts by weight of the base oil. All the above can be performance enhanced using a variety of cobase stocks, AN, AB, ADPO, ADPS, ADPM, and/or a variety of mono-basic, di-basic, and tribasic esters in conjunction with low sulfur, low aromatic, low iodine number, low bromine number, high aniline point, isoparafin.

## EXAMPLES

## Example 1

In this example, we formulated an embodiment of the inventive gear oil to compare to a standard commercially available gear oil. The amount of each base oil and relative amounts of specific additives are shown for the two blends. The two blends were formulated to have the same base stock amounts with the only difference being the additive. The specific additives are listed for the inventive embodiment with the commercially available gear oil using a standard high sulfur gear oil package. The two blends were formulated for an ISO 320 viscosity gear oil shown in table 8.

TABLE 8

|                           |                                       | Inventive Example 1 | Comparative Example 2 |
|---------------------------|---------------------------------------|---------------------|-----------------------|
| <u>Identification</u>     |                                       |                     |                       |
| High Viscosity Base oil   | PAO 150                               | 40.00               | 40.00                 |
| High Viscosity Base oil   | PAO 100                               | 30.19               | 30.19                 |
| Low Viscosity Base oil    | PAO 4                                 | 15.91               | 15.91                 |
| Low Viscosity Co-Base oil | Ester, Alkylated Aromatic or mixtures | 12.00               | 12.00                 |
| <u>Additive Function</u>  |                                       |                     |                       |
| Antiwear system           | Phosphate                             | 0.30                | —                     |
| Rust Inhibitors           | Alkylated Acid type                   | 0.40                | —                     |
| Friction Modifier         | Phosphate                             | 0.25                | —                     |
| Metal Passivator          | Phosphate                             | 0.10                | —                     |
| Antioxidant               | Amine                                 | 0.40                | —                     |
| Defoamant/Demulsifier     | AF pkg                                | 0.40                | —                     |
| Hi S-Gear oil package     | S-containing AW pkg                   | —                   | 2.65                  |

42

TABLE 9

| Comparative Data                        | Inventive Example 1 | Comparative Example 2 |
|-----------------------------------------|---------------------|-----------------------|
| FVA 54 Micropitting, Profile Deviation  | 6.1 microns         | 8.2 microns           |
| FZG Skuffing A/8.3/90, FLS              | 14+                 | 13                    |
| D3427, air release @ 75 C.              | 5.3 mins            | 8.3 mins              |
| D130, Copper Strip test, 121 C., 24 hrs | 1B                  | 3B                    |

5

10

As shown in table 9, the inventive blend provides superior micropitting, wear scuffing, air release and corrosion properties when compared to the standard high sulfur gear oil even when the same base stock combinations are used.

A SWGR worm gear efficiency and operating temperature test was run on the blends. Table 10 shows the significant benefit of worm gear efficiency and operating temperature in using the additive package in the preferred base stock combinations. FIG. 3 is a bar graph of the worm gear efficiency of the inventive example 1 (line 31) and the comparative example 2 (line 35). FIG. 4 is a bar graph of the operating temperature of the inventive example 1 (line 41) and the comparative example 2 (line 45).

TABLE 10

|                       | Worm Gear Efficiency %, | Operating Temp, (° F.) |
|-----------------------|-------------------------|------------------------|
| Inventive Example A   | 76.3                    | 169.2                  |
| Comparative Example B | 73.6                    | 183.2                  |

## Example 2

40 A second set of comparative sample were formulated to further demonstrate the synergistic benefits of combining the inventive additive system with the preferred base stock combination. As shown in Table 11, all the formulations were blended with high viscosity PAO base stock to create an 45 extreme modal blend. The same base stocks combinations were then compared using an embodiment of the inventive additive package versus a commercially available high sulfur gear oil package.

TABLE 11

| Base stock Component | Blend: |       |      |       |       |       |
|----------------------|--------|-------|------|-------|-------|-------|
|                      | A      | B     | C    | D     | E     | F     |
| ISO                  | 460    | 460   | 320  | 320   | 320   | 320   |
| Adipate Ester        | —      | —     | —    | —     | —     | —     |
| TMP Ester            | 10     | 10    | 10   | 10    | 10    | 10    |
| PAO 2 cSt            | —      | —     | —    | —     | —     | —     |
| PAO 4 cSt            | 14     | 14    | 18   | 18    | 18    | 18    |
| PAO 6 cSt            | —      | —     | —    | —     | —     | —     |
| PAO 100 cSt          | —      | —     | —    | 34.1  | 34.15 | 34.15 |
| PAO 150 cSt          | 73.1   | 73.15 | 69.1 | 69.15 | 35    | 35    |

TABLE 11-continued

| Additive Component     | Blend:                    |       |                           |     |                           |      |
|------------------------|---------------------------|-------|---------------------------|-----|---------------------------|------|
|                        | A                         | B     | C                         | D   | E                         | F    |
|                        | % in Additive Concentrate |       | % in Additive Concentrate |     | % in Additive Concentrate |      |
| Antiwear               | 1.2                       | 41.3  | —                         | 1.2 | 41.3                      | —    |
| Antirust               | 0.3                       | 10.4  | —                         | 0.3 | 10.4                      | —    |
| Metal passivator       | 0.1                       | 3.5   | —                         | 0.1 | 3.5                       | —    |
| Antioxidant            | 0.4                       | 13.8  | —                         | 0.4 | 13.8                      | —    |
| Friction modifier      | 0.7                       | 24.1  | —                         | 0.7 | 24.1                      | —    |
| Hi S-Gear oil package  | —                         | —     | 2.65                      | —   | —                         | 2.65 |
| Defoamant              | 0.2                       | 6.9   | —                         | 0.2 | 6.9                       | —    |
| Total Additive Treat % | 2.9                       | 100.0 | 2.65                      | 2.9 | 100.0                     | 2.65 |

20

Table 11 shows the formulations of the three novel blends relative to the three blends with the high sulfur gear oil package. As shown in Table 12 Examples A, C, and E all have superior properties when compared to their corresponding Examples B, D, and F respectively. These properties include corrosion, oxidation and flash points.

In another embodiment, another benefit of the improved base stocks properties is the ability to use less additives. In a preferred embodiment, the base stock combination provides the ability to use treat rates preferably less than 10 percent and even more preferably less than 5 percent.

TABLE 12

|                                               | Blend |      |      |      |      |      |
|-----------------------------------------------|-------|------|------|------|------|------|
|                                               | A     | B    | C    | D    | E    | F    |
| ASTM D 130 Copper Corrosion                   | 1B    | 3B   | 1A   | 3B   | 1B   | 3E   |
| ASTM D665B Synthetic Sea Water Corr. On Steel | Pass  | Fail | Pass | Fail | Pass | Fail |
| ASTM D2272 Rotary Bomb Oxidation Test         | 1082  | 74   | 1138 | 77   | 1103 | 86   |
| ASTM D92 Flash Point (° C.)                   | 247   | 226  | 250  | 230  | 248  | 221  |
| ASTM D2893 Oxidation Test - EOT A TAN Inc.    | 0.10  | 1.28 | 0.25 | 1.61 | 0.15 | 2.59 |

40

While the examples have been to gear oils, these examples are not intended to be limiting. The novel formulations provide improved properties of all lubricating uses including but not limited to industrial and hydraulic oils.

In addition, based on the disclosure herein other base stocks of widely disparate viscosities that give a “bi-modal” or “extreme-modal” blending result can also be envisioned with the benefit of the disclosure herein to deliver favorable lubricating properties. These properties include but are not limited to micropitting, air release, pour point, low temperature viscosity, pour point, shear stability, and any combination thereof. While the benefits discussed herein are primarily for the use of gear oil, the benefits would apply to all lubricants including marine, automotive, and industrial. The claims are intended to include all suitable lubricant applications.

In one embodiment, no VI improvers are needed due to the high inherent VI of the base stocks. This benefit permits the ability to avoid VI improvers that may adversely affect shear stability. In this embodiment, the shear stability of the lubricant should be less than 15 percent and even more preferably less than 10 percent and in the most preferred embodiment, there will be essentially no VI improvers.

In a preferred embodiment, no transition or alkali metals are used in the finished formulation. This finished formulation would provide enhanced hydrolytic stability.

45

What is claimed is:

1. A gear and bearing oil, comprising
    - a) at least three base stocks;
    - b) a first PAO base stock with a viscosity at least 100 cSt, Kv100° C.;
    - c) a second base stock comprising a oil with a viscosity less than 40 cSt, Kv100° C.;
    - d) a third basestock comprising a co-base oil selected from the group consisting of a PAO with a viscosity of at least 1.5 cSt, Kv100° C. and no more than 100 cSt, Kv100° C., a Group V base stock including ester base stock, alkylated aromatic and any combination thereof;
    - e) an additive package comprising at least one antiwear additive, at least one antioxidant additive, at least one rust inhibitor additive, at least one metal passivator additive, at least one demulsifier additive, at least one defoamant additive with the proviso that the additive package does not include any sulfur containing and any metallic containing additives;
- wherein the antiwear additive is at least 0.05 and less than 1 weight percent of the final formulation the antioxidant additive is at least 0.05 and less than 0.5 weight percent of the final formulation, the rust inhibitor additive is at least 0.05 and less than 0.5 weight percent of the final formulation, the metal passivator additive is at least 0.01 and less than 0.5 weight percent of the final formulation,

50

55

60

65

**45**

the demulsifier additive is at least 0.05 and less than 1 weight percent of the final formulation, and the defoamant additive is at least 0.005 and less than 1 weight percent of the final formulation;

f) wherein the gear and bearing oil has less than 1000 ppm phosphorous, less than 500 ppm nitrogen, less than 10 ppm metals, less than 30 ppm sulfur and a TAN of less than 1.

2. The gear and bearing oil of claim 1 further including at least one friction modifier additive.

3. The gear and bearing oil of claim 2 wherein the antiwear additive is a phosphate or amine phosphate, the rust inhibitor additive is an alkylated acid type, the friction modifier additive is a phosphonate, the metal passivator additive is an amine phosphate and the defoamant additive is an antifoam package having a demulsifier additive.

4. The gear and bearing oil of claim 3 wherein the gear and bearing oil has a treat rate of less than 10 percent.

5. The gear and bearing oil of claim 1 wherein the second base stock is chosen from the group consisting of GTL base stock, wax derived base stock, Poly-Alpha-Olefin (PAO), Brightstocks, Brightstocks with PIB, Group I base stocks, Group II base stocks, Group III base stocks, Group V base stocks, Group VI base stocks, and any combination thereof.

6. The gear and bearing oil of claim 1 wherein the first base stock has a molecular weight distribution less than algorithm:

$$MWD=0.41667+0.725\log(Kv \text{ at } 100^\circ \text{ C. in cSt}).$$

7. The gear and bearing oil of claim 6 wherein the first base PAO stock is a metallocene catalyzed PAO.

8. A method of obtaining favorable gear and bearing oil properties, comprising:

a) obtaining a first PAO base stock having a viscosity greater than 100 cSt, Kv100° C and having a molecular weight distribution (MWD) as a function of viscosity at least 10 percent less than algorithm

$$MWD=0.2223+1.0232\log(Kv \text{ at } 100^\circ \text{ C in cSt});$$

**46**

b) obtaining a second base stock lubricant, the second base stock lubricant has a viscosity less than 40 cSt, Kv100° C;

c) obtaining an additive package comprising at least one antiwear additive, at least one antioxidant additive, at least one rust inhibitor additive, at least one metal passivator additive, at least one demulsifier additive, at least one defoamant additive with the proviso that the additive package does not include any sulfur containing and any metallic containing additives;

wherein the antiwear additive is at least 0.05 and less than 1 weight percent of the final formulation, the antioxidant additive is at least 0.05 and less than 0.5 weight percent of the final formulation, the rust inhibitor additive is at least 0.05 and less than 0.5 weight percent of the final formulation, the metal passivator additive is at least 0.01 and less than 0.5 weight percent of the final formulation, the demulsifier additive is at least 0.05 and less than 1 weight percent of the final formulation, and the defoamant additive is at least 0.005 and less than 1 weight percent of the final formulation;

d) blending the first base stock, the second base stock and additive package to produce a gear and bearing oil wherein the gear and bearing oil has less than 1000 ppm phosphorous, less than 500 ppm nitrogen, less than 10 ppm metals, less than 30 ppm sulfur and a TAN of less than 1.

9. The gear and bearing oil of claim 8 further including at least one friction modifier additive.

10. The gear and bearing oil of claim 9 wherein the antiwear additive is a phosphate or amine phosphate, the rust inhibitor is an alkylated acid type, the friction modifier is a phosphonate, the metal passivator is an amine phosphate and the defoamant is an antifoam package having a demulsifier additive.

11. The gear and bearing oil of claim 8 wherein the first PAO base stock is a metallocene catalyzed PAO.

\* \* \* \* \*